



US007074537B2

(12) **United States Patent**  
**Qian et al.**

(10) **Patent No.:** **US 7,074,537 B2**  
(b5) **Date of Patent:** **Jul. 11, 2006**

(54) **ORGANOSOL LIQUID TONER INCLUDING AMPHIPATHIC COPOLYMERIC BINDER HAVING CRYSTALLINE COMPONENT**

(75) Inventors: **Julie Y. Qian**, Woodbury, MN (US); **Gay L. Herman**, Cottage Grove, MN (US); **James A. Baker**, Hudson, WI (US)

(73) Assignee: **Samsung Electronics Company**, Suwon (KR)

(\*) Notice: Subject to any disclaimer, the term of this patent is extended or adjusted under 35 U.S.C. 154(b) by 67 days.

(21) Appl. No.: **10/612,534**

(22) Filed: **Jun. 30, 2003**

(65) **Prior Publication Data**

US 2004/0091808 A1 May 13, 2004

**Related U.S. Application Data**

(60) Provisional application No. 60/425,515, filed on Nov. 12, 2002.

(51) **Int. Cl.**  
**G03G 9/13** (2006.01)

(52) **U.S. Cl.** ..... **430/114**; 430/137.22; 430/115; 430/117

(58) **Field of Classification Search** ..... 430/114, 430/115, 117, 137.22

See application file for complete search history.

(56) **References Cited**

**U.S. PATENT DOCUMENTS**

|               |         |                 |       |         |
|---------------|---------|-----------------|-------|---------|
| 3,411,936 A   | 11/1968 | Roteman et al.  | ..... | 117/37  |
| 4,268,598 A   | 5/1981  | Leseman et al.  | ..... | 430/107 |
| 4,321,404 A   | 3/1982  | Williams et al. | ..... | 560/115 |
| 4,476,210 A   | 10/1984 | Croucher et al. | ..... | 430/114 |
| 4,613,559 A   | 9/1986  | Ober et al.     | ..... | 430/137 |
| 4,727,011 A   | 2/1988  | Mahabadi et al. | ..... | 430/138 |
| 4,728,983 A   | 3/1988  | Zwadlo et al.   | ..... | 355/4   |
| 4,762,764 A   | 8/1988  | Ng et al.       | ..... | 430/115 |
| 4,794,651 A   | 12/1988 | Landa et al.    | ..... | 430/110 |
| 4,925,766 A   | 5/1990  | Elmasry et al.  | ..... |         |
| 4,937,167 A   | 6/1990  | Moffat et al.   | ..... | 430/137 |
| 4,965,161 A   | 10/1990 | Mahmud          | ..... | 430/109 |
| 4,978,598 A   | 12/1990 | Elmasry et al.  | ..... | 430/137 |
| 5,023,159 A   | 6/1991  | Ong et al.      | ..... | 430/109 |
| 5,061,587 A   | 10/1991 | Tsubuko et al.  | ..... | 430/109 |
| 5,115,277 A   | 5/1992  | Camis           | ..... | 355/273 |
| 5,262,259 A   | 11/1993 | Chou et al.     | ..... | 430/47  |
| 5,264,315 A   | 11/1993 | Tan et al.      | ..... | 430/137 |
| 5,384,226 A   | 1/1995  | Kanakura et al. | ..... | 430/137 |
| 5,410,392 A   | 4/1995  | Landa           | ..... | 355/271 |
| 5,482,809 A   | 1/1996  | Rao et al.      | ..... |         |
| 5,529,873 A   | 6/1996  | Chiba et al.    | ..... | 430/109 |
| 5,650,253 A   | 7/1997  | Baker et al.    | ..... | 430/119 |
| 5,652,282 A   | 7/1997  | Baker et al.    | ..... | 523/201 |
| 5,698,616 A   | 12/1997 | Baker et al.    | ..... | 523/201 |
| 5,886,067 A * | 3/1999  | Li et al.       | ..... | 523/201 |
| 5,916,718 A   | 6/1999  | Kellie et al.   | ..... | 430/45  |
| 5,965,314 A   | 10/1999 | Herman et al.   | ..... | 430/126 |

|                 |         |                  |       |            |
|-----------------|---------|------------------|-------|------------|
| 6,037,090 A     | 3/2000  | Tanaka et al.    | ..... | 430/106    |
| 6,088,560 A     | 7/2000  | Zenk et al.      | ..... | 399/237    |
| 6,102,526 A     | 8/2000  | Tunius           | ..... | 347/55     |
| 6,103,781 A     | 8/2000  | Li et al.        | ..... | 523/201    |
| 6,136,490 A     | 10/2000 | Ogawa et al.     | ..... | 430/109    |
| 6,210,852 B1    | 4/2001  | Nakamura         | ..... | 430/110    |
| 6,221,545 B1    | 4/2001  | Tran et al.      | ..... | 430/10     |
| 6,248,494 B1    | 6/2001  | Yamazaki et al.  | ..... | 430/110    |
| 6,255,363 B1    | 7/2001  | Baker et al.     | ..... | 523/201    |
| 6,316,157 B1    | 11/2001 | Yoshikawa et al. | ..... | 430/110    |
| 6,352,810 B1    | 3/2002  | Jiang et al.     | ..... | 430/137.11 |
| 6,475,685 B1    | 11/2002 | Uchida et al.    | ..... | 430/99     |
| 6,546,221 B1    | 4/2003  | Baker et al.     | ..... | 399/237    |
| 6,647,234 B1    | 11/2003 | Herman et al.    | ..... | 399/238    |
| 6,649,316 B1 *  | 11/2003 | Baker et al.     | ..... | 430/114    |
| 2002/0128349 A1 | 9/2002  | Qian et al.      | ..... |            |
| 2004/0024090 A1 | 2/2004  | Suda et al.      | ..... |            |

**FOREIGN PATENT DOCUMENTS**

|    |               |         |
|----|---------------|---------|
| EP | 1229057 A2    | 8/2002  |
| EP | 1251406 A2    | 10/2002 |
| JP | 05-119529     | 5/1993  |
| JP | 2004-035736   | 5/2004  |
| WO | WO 92/17825   | 10/1992 |
| WO | WO97/12284    | 4/1997  |
| WO | WO98/24002    | 6/1998  |
| WO | WO01/79318 A1 | 10/2001 |
| WO | WO01/79363 A2 | 10/2001 |
| WO | WO01/79364 A2 | 10/2001 |

**OTHER PUBLICATIONS**

Copy of European Search Report for EP1420305 A1 issued on Mar. 15, 2004, 2 pgs.

U.S. Appl. No. 10/612,243, filed Jun. 30, 2003, entitled "Organosol Including Amphipathic Copolymeric Binder and Use of the Organosol to Make Dry Toners for Electrographic Applications" (30 pgs.).

U.S. Appl. No. 10/612,535, filed Jun. 30, 2003, entitled "Organosol Including Amphipathic Copolymeric Binder Having Crystalline Material, and Use of the Organosol to Make Dry Toners for Electrographic Applications" (32 pgs.).

(Continued)

*Primary Examiner*—John L Goodrow

(74) *Attorney, Agent, or Firm*—Kagan Binder, PLLC

(57) **ABSTRACT**

Liquid electrographic toners are derived from organosols incorporating amphipathic copolymeric binder particles that include polymerizable, crystallizable compounds chemically incorporated into the dispersed portion of the copolymer. The invention further provides organosols that include amphipathic copolymeric binder particles that include a dispersed (D) portion and a solvated (S) portion, wherein the D portion has a high glass transition temperature, and at least one polymerizable, crystallizable compound is chemically incorporated into the D portion, the S portion, or both the D and S portion of the copolymer. Methods of making and electrographically printing liquid toners derived from these organosols are also described. The invention is particularly suited for preparing liquid toners for electrophotographic printing.

OTHER PUBLICATIONS

U.S. Appl. No. 10/612,765, filed Jun. 30, 2003, entitled "Organosol Including High Tg Amphipathic Copolymeric Binder and Liquid Toners for Electrophotographic Applications" (26 pgs.).

U.S. Appl. No. 10/612,533, filed Jun. 30, 2003, entitled "Organosol Including Amphipathic Copolymeric Binder Made with Soluble High Tg Monomer and Liquid Toners for Electrophotographic Applications" (29 pgs.).

\* cited by examiner

**ORGANOSOL LIQUID TONER INCLUDING  
AMPHIPATHIC COPOLYMERIC BINDER  
HAVING CRYSTALLINE COMPONENT**

This application claims the benefit of U.S. Provisional Application Ser. No. 60/425,515, filed Nov. 12, 2002, entitled "ORGANOSOL LIQUID TONER INCLUDING AMPHIPATHIC COPOLYMERIC BINDER HAVING CRYSTALLINE COMPONENT," now lapsed, which application is incorporated herein by reference in its entirety.

**FIELD OF THE INVENTION**

The present invention relates to liquid toner compositions having utility in electrography. More particularly, the invention relates liquid electrophotographic toners derived from organosols incorporating amphipathic copolymeric binder particles that include polymerizable, crystallizable compounds chemically incorporated into the dispersed portion of the copolymeric binder. The invention further relates to organosols incorporating amphipathic copolymeric binder particles that include one or more dispersed (D) portions and one or more solvated (S) portions, wherein one or more of the D portions has a high glass transition temperature, and at least one polymerizable, crystallizable compound is chemically incorporated into the D portion, the S portion, or both the D portion and S portion of the copolymer.

**BACKGROUND OF THE INVENTION**

In electrophotographic and electrostatic printing processes (collectively electrographic processes), an electrostatic image is formed on the surface of a photoreceptive element or dielectric element, respectively. The photoreceptive element or dielectric element may be an intermediate transfer drum or belt or the substrate for the final toned image itself, as described by Schmidt, S. P. and Larson, J. R. in *Handbook of Imaging Materials* Diamond, A. S., Ed: Marcel Dekker, New York; Chapter 6, pp 227-252, and U.S. Pat. Nos. 4,728,983, 4,321,404, and 4,268,598.

In electrostatic printing, a latent image is typically formed by (1) placing a charge image onto a dielectric element (typically the receiving substrate) in selected areas of the element with an electrostatic writing stylus or its equivalent to form a charge image, (2) applying toner to the charge image, and (3) fixing the toned image. An example of this type of process is described in U.S. Pat. No. 5,262,259.

In electrophotographic printing, also referred to as xerography, electrophotographic technology is used to produce images on a final image receptor, such as paper, film, or the like. Electrophotographic technology is incorporated into a wide range of equipment including photocopiers, laser printers, facsimile machines, and the like.

Electrophotography typically involves the use of a reusable, light sensitive, temporary image receptor, known as a photoreceptor, in the process of producing an electrophotographic image on a final, permanent image receptor. A representative electrophotographic process involves a series of steps to produce an image on a receptor, including charging, exposure, development, transfer, fusing, and cleaning, and erasure.

In the charging step, a photoreceptor is covered with charge of a desired polarity, either negative or positive, typically with a corona or charging roller. In the exposure step, an optical system, typically a laser scanner or diode array, forms a latent image by selectively discharging the charged surface of the photoreceptor in an imagewise man-

ner corresponding to the desired image to be formed on the final image receptor. In the development step, toner particles of the appropriate polarity are generally brought into contact with the latent image on the photoreceptor, typically using a developer electrically-biased to a potential opposite in polarity to the toner polarity. The toner particles migrate to the photoreceptor and selectively adhere to the latent image via electrostatic forces, forming a toned image on the photoreceptor.

10 In the transfer step, the toned image is transferred from the photoreceptor to the desired final image receptor; an intermediate transfer element is sometimes used to effect transfer of the toned image from the photoreceptor with subsequent transfer of the toned image to a final image receptor. In the fusing step, the toned image on the final image receptor is heated to soften or melt the toner particles, thereby fusing the toned image to the final receptor. An alternative fusing method involves fixing the toner to the final receptor under high pressure with or without heat. In 15 the cleaning step, residual toner remaining on the photoreceptor is removed.

Finally, in the erasing step, the photoreceptor charge is reduced to a substantially uniformly low value by exposure to light of a particular wavelength band, thereby removing 20 remnants of the original latent image and preparing the photoreceptor for the next imaging cycle.

Two types of toner are in widespread, commercial use: liquid toner and dry toner. The term "dry" does not mean that the dry toner is totally free of any liquid constituents, but 25 connotes that the toner particles do not contain any significant amount of solvent, e.g., typically less than 10 weight percent solvent (generally, dry toner is as dry as is reasonably practical in terms of solvent content), and are capable of carrying a triboelectric charge. This distinguishes dry toner particles from liquid toner particles.

A typical liquid toner composition generally includes toner particles suspended or dispersed in a liquid carrier. The liquid carrier is typically nonconductive dispersant, to avoid discharging the latent electrostatic image. Liquid toner particles are generally solvated to some degree in the liquid carrier (or carrier liquid), typically in more than 50 weight percent of a low polarity, low dielectric constant, substantially nonaqueous carrier solvent. Liquid toner particles are also typically smaller than dry toner particles. Because of 35 their small particle size, ranging from about 5 microns to sub-micron, liquid toners are capable of producing very high-resolution toned images.

A typical toner particle for a liquid toner composition generally comprises a copolymeric binder and optionally 50 one or more visual enhancement additives (for example, a colored pigment particle). The polymeric binder fulfills functions both during and after the electrophotographic process. With respect to processability, the character of the binder impacts charging and charge stability, flow, and 55 fusing characteristics of the toner particles. These characteristics are important to achieve good performance during development, transfer, and fusing. After an image is formed on the final receptor, the nature of the binder (e.g. glass transition temperature, melt viscosity, molecular weight) and the fusing conditions (e.g. temperature, pressure and fuser configuration) impact durability (e.g. blocking and erasure resistance), adhesion to the receptor, gloss, and the like.

Polymeric binder materials suitable for use in liquid toner 60 particles typically exhibit glass transition temperatures of about -24° C. to 55° C., which is lower than the range of glass transition temperatures (50-100° C.) typical for poly-

meric binders used in dry toner particles. In particular, some liquid toners are known to incorporate polymeric binders exhibiting glass transition temperatures ( $T_g$ ) below room temperature (25° C.) in order to rapidly self fix, e.g. by film formation, in the liquid electrophotographic imaging process; see e.g. U.S. Pat. No. 6,255,363. However, such liquid toners are also known to exhibit inferior image durability resulting from the low  $T_g$  (e.g. poor blocking and erasure resistance) after fusing the toned image to a final image receptor.

To overcome these durability deficiencies, polymeric materials selected for use in dry toners more typically exhibit a range of  $T_g$  of at least about 55–65° C. in order to obtain good blocking resistance after fusing, yet typically require high fusing temperatures of about 200–250° C. in order to soften or melt the toner particles and thereby adequately fuse the toner to the final image receptor. High fusing temperatures are a disadvantage for dry toners because of the long warm-up time and higher energy consumption associated with high temperature fusing and because of the risk of fire associated with fusing toner to paper at temperatures approaching the autoignition temperature of paper (233° C.).

Although some liquid toners are known to use higher  $T_g$  (greater than or equal to about 60° C.) polymeric binders, such toners are known to exhibit other problems related to the choice of polymeric binder, including image defects due to the inability of the liquid toner to rapidly self fix in the imaging process, poor charging and charge stability, poor stability with respect to agglomeration or aggregation in storage, poor sedimentation stability in storage, and the requirement that high fusing temperatures of about 200–250° C. be used in order to soften or melt the toner particles and thereby adequately fuse the toner to the final image receptor.

In addition, some liquid and dry toners using high  $T_g$  polymeric binders are known to exhibit undesirable partial transfer (offset) of the toned image from the final image receptor to the fuser surface at temperatures above or below the optimal fusing temperature, requiring the use of low surface energy materials in the fuser surface or the application of fuser oils to prevent offset. Alternatively, various lubricants or waxes have been physically blended into the dry toner particles during fabrication to act as release or slip agents; however, because these waxes are not chemically bonded to the polymeric binder, they may adversely affect triboelectric charging of the toner particle or may migrate from the toner particle and contaminate the photoreceptor, an intermediate transfer element, the fuser element, or other surfaces critical to the electrophotographic process.

In addition to the polymeric binder and the optional visual enhancement additive, liquid toner compositions can optionally include other additives. For example, charge control agents can be added to impart an electrostatic charge on the toner particles. Dispersing agents can be added to provide colloidal stability, aid fixing of the image, and provide charged or charging sites for the particle surface. Dispersing agents are commonly added to liquid toner compositions because toner particle concentrations are high (inter-particle distances are small) and electrical double-layer effects alone will not adequately stabilize the dispersion with respect to aggregation or agglomeration. Release agents can also be used to help prevent the toner from sticking to fuser rolls when those are used. Other additives include antioxidants, ultraviolet stabilizers, fungicides, bactericides, flow control agents, and the like.

One fabrication technique involves synthesizing an amphiphilic copolymeric binder dispersed in a liquid carrier to form an organosol, then mixing the formed organosol with other ingredients to form a liquid toner composition. 5 Typically, organosols are synthesized by nonaqueous dispersion polymerization of polymerizable compounds (e.g. monomers) to form copolymeric binder particles that are dispersed in a low dielectric hydrocarbon solvent (carrier liquid). These dispersed copolymer particles are sterically-10 stabilized with respect to aggregation by chemical bonding of a steric stabilizer (e.g. graft stabilizer), solvated by the carrier liquid, to the dispersed core particles as they are formed in the polymerization. Details of the mechanism of such steric stabilization are described in Napper, D. H., 15 "Polymeric Stabilization of Colloidal Dispersions," Academic Press, New York, N.Y., 1983. Procedures for synthesizing self-stable organosols are described in "Dispersion Polymerization in Organic Media," K. E. J. Barrett, ed., John Wiley: New York, N.Y., 1975. Liquid toner compositions 20 have been manufactured using dispersion polymerization in low polarity, low dielectric constant carrier solvents for use in making relatively low glass transition temperature ( $T_g \leq 30$ ° C.) film-forming liquid toners that undergo rapid self-fixing in the electrophotographic imaging process. See, e.g., U.S. Pat. Nos. 5,886,067 and 6,103,781. Organosols 25 have also been prepared for use in making intermediate glass transition temperature ( $T_g$  between 30–55° C.) liquid electrostatic toners for use in electrostatic stylus printers. See e.g. U.S. Pat. No. 6,255,363 B1. A representative non-30 aqueous dispersion polymerization method for forming an organosol is a free radical polymerization carried out when one or more ethylenically-unsaturated monomers, soluble in a hydrocarbon medium, are polymerized in the presence of a preformed, polymerizable solution polymer (e.g. a graft 35 stabilizer or "living" polymer). See U.S. Pat. No. 6,255,363.

Once the organosol has been formed, one or more additives can be incorporated, as desired. For example, one or 40 more visual enhancement additives and/or charge control agents can be incorporated. The composition can then subjected to one or more mixing processes, such as homogenization, microfluidization, ball-milling, attritor milling, high energy bead (sand) milling, basket milling or other techniques known in the art to reduce particle size in a dispersion. The mixing process acts to break down aggregated 45 visual enhancement additive particles, when present, into primary particles (having a diameter in the range of 0.05 to 1.0 microns) and may also partially shred the dispersed copolymeric binder into fragments that can associate with the surface of the visual enhancement additive.

50 According to this embodiment, the dispersed copolymer or fragments derived from the copolymer then associate with the visual enhancement additive, for example, by adsorbing to or adhering to the surface of the visual enhancement additive, thereby forming toner particles. The result is a sterically-stabilized, nonaqueous dispersion of toner particles having a size in the range of about 0.1 to 2.0 microns, with typical toner particle diameters in the range 0.1 to 0.5 microns. In some embodiments, one or more charge control agents can be added after mixing, if desired.

55 Several characteristics of liquid toner compositions are important to provide high quality images. Toner particle size and charge characteristics are especially important to form high quality images with good resolution. Further, rapid self-fixing of the toner particles is an important requirement 60 for some liquid electrophotographic printing applications, e.g. to avoid printing defects (such as smearing or trailing-edge tailing) and incomplete transfer in high-speed printing.

Another important consideration in formulating a liquid toner composition relates to the durability and archivability of the image on the final receptor. Erasure resistance, e.g. resistance to removal or damage of the toned image by abrasion, particularly by abrasion from natural or synthetic rubber erasers commonly used to remove extraneous pencil or pen markings, is a desirable characteristic of liquid toner particles.

Resistance of the image on the final image receptor to damage by blocking to the receptor (or to other toned surfaces) is another desirable characteristic of liquid toner particles. Therefore, another important consideration in formulating a liquid toner is the tack of the image on the final receptor. It is desirable for the image on the final receptor material to be essentially tack-free over a fairly wide range of temperatures. If the image has a residual tack, then the image can become embossed or picked off when placed in contact with another surface (also referred to as blocking). This is particularly a problem when printed sheets are placed in a stack.

To address this concern, a film laminate or protective layer may be placed over the surface of the image. This laminate often acts to increase the effective dot gain of the image, thereby interfering with the color rendition of a color composite. In addition, lamination of a protective layer over a final image surface adds both extra cost of materials and extra process steps to apply the protective layer, and may be unacceptable for certain printing applications (e.g. plain paper copying or printing).

Another method to improve the durability of liquid toned images and address the drawbacks of lamination is described in U.S. Pat. No. 6,103,781. U.S. Pat. No. 6,103,781 describes a liquid ink composition containing organosols having side-chain or main-chain crystallizable polymeric moieties. At column 6, lines 53–60, the authors describe a binder resin that is an amphipathic copolymer dispersed in a liquid carrier (also known as an organosol) that includes a high molecular weight (co)polymeric steric stabilizer covalently bonded to an insoluble, thermoplastic (co)polymeric core. The steric stabilizer includes a crystallizable polymeric moiety that is capable of independently and reversibly crystallizing at or above room temperature (22° C.).

According to the authors, superior stability of the dispersed toner particles with respect to aggregation is obtained when at least one of the polymers or copolymers (denoted as the stabilizer) is an amphipathic substance containing at least one oligomeric or polymeric component having a weight-average molecular weight of at least 5,000 that is solvated by the liquid carrier. In other words, the selected stabilizer, if present as an independent molecule, would have some finite solubility in the liquid carrier. Generally, this requirement is met if the absolute difference in Hildebrand solubility parameter between the steric stabilizer and the solvent is less than or equal to 3.0 MPa<sup>1/2</sup>.

As described in U.S. Pat. No. 6,103,781, the composition of the insoluble resin core is preferentially manipulated such that the organosol exhibits an effective glass transition temperature ( $T_g$ ) of less than 22° C., more preferably less than 6° C. Controlling the glass transition temperature allows one to formulate an ink composition containing the resin as a major component to undergo rapid film formation (rapid self-fixing) in liquid electrophotographic printing or imaging processes using offset transfer processes carried out at temperatures greater than the core  $T_g$ , preferably at or above 22° C. (Column 10, lines 36–46).

## SUMMARY OF THE INVENTION

The present invention relates to liquid toner compositions having utility in electrophotography. In particular, the present invention relates to liquid toner compositions comprising organosols incorporating amphipathic copolymers having crystalline polymer material incorporated into the dispersed portion of the amphipathic copolymer. The organosol is easily combined with additional ingredients, such as one or more visual enhancement additives and other desired ingredients, and subjected to mixing processes to form a liquid toner composition.

In one embodiment, the invention relates to organosols incorporating amphipathic copolymeric binder particles that include one or more dispersed (D) portions and one or more solvated (S) portions, wherein one or more polymerizable, crystallizable compounds are chemically incorporated into the dispersed portion of the amphipathic copolymer. In some embodiments, the invention relates to organosols incorporating amphipathic copolymeric binder particles, wherein the D portion has a high glass transition temperature ( $T_g$ , above about 55° C.) and at least one polymerizable, crystallizable compound is chemically incorporated into the D portion, the S portion, or both the D portion and S portion of the copolymer. In other embodiments, the invention relates to organosols incorporating amphipathic copolymeric binder particles, wherein the D portion has a glass transition temperature in the range of 30° C. to 50° C., and at least one polymerizable, crystallizable compound is chemically incorporated into the D portion, the S portion, or both the D portion and the S portion of the copolymer.

The toner particles of the liquid toner composition advantageously include a polymeric binder that comprises an amphipathic copolymer, and optionally at least one visual enhancement additive, for example, a colorant particle. As used herein, the term "amphipathic" refers to a copolymer having a combination of portions having distinct solubility and dispersibility characteristics in a desired liquid carrier that is used to make the copolymer and/or used in the course of preparing the liquid toner particles. Preferably, the liquid carrier is selected such that at least one portion (also referred to herein as S material or portion(s)) of the copolymer is more solvated by the carrier while at least one other portion (also referred to herein as D material or portion(s)) of the copolymer constitutes more of a dispersed phase in the carrier.

In preferred embodiments, the copolymer is polymerized in situ in the desired liquid carrier as this yields substantially monodisperse copolymeric particles suitable for use in liquid toner compositions with little, if any, need for subsequent comminuting or classifying. The resulting organosol is then preferably converted into toner particles by mixing the organosol with other optional ingredients, such as at least one visual enhancement additive and other desired ingredients. During such combination, ingredients comprising the visual enhancement particles and the amphipathic copolymer will tend to self-assemble into composite toner particles. Specifically, it is believed that the D portion of the copolymer will tend to physically and/or chemically interact with the surface of the visual enhancement additive, while the S portion helps promote dispersion in the carrier without use of a separate surfactant or dispersant.

Additionally, a wide range of liquid carrier soluble or dispersible monomers may be used to form the organosol by a variety of substantially nonaqueous polymerization methods. Preferably, substantially nonaqueous dispersion polymerization is used to polymerize monomers using free

radical polymerization methods as desired. As used herein, "substantially nonaqueous polymerization methods" refers to polymerization methods in an organic solvent containing at most a minor portion of water.

In certain embodiments, the dispersed amphipathic copolymer particles comprises at least one portion comprising crystalline material derived from ingredients comprising one or more polymerizable crystallizable compounds (PCC's), for example, one or more crystalline monomers that are chemically incorporated into the D portion. In some preferred embodiments, the organosol incorporates amphipathic copolymeric binder particles that include polymerizable, crystallizable compounds chemically incorporated into the dispersed portion of the copolymer. In other preferred embodiments, the organosol incorporates amphipathic copolymeric binder particles that include a dispersed (D) portion and a solvated (S) portion, wherein the D portion has a high glass transition temperature ( $T_g$  greater than about 55° C.), and at least one polymerizable, crystallizable compound is chemically incorporated into the D portion, the S portion, or both the D and S portions of the copolymer. In other preferred embodiments, the organosol incorporates amphipathic copolymeric binder particles that include a dispersed (D) portion and a solvated (S) portion, wherein the D portion has a glass transition temperature in the range of about 30° C. to 50° C., and at least one polymerizable, crystallizable compound is chemically incorporated into the D portion, the S portion, or both the D and S portions of the copolymer.

Suitable PCC's include monomers, functional oligomers, functional pre-polymers, macromers or other compounds able to undergo polymerization to form a polymer, wherein at least a portion of the polymer is capable of undergoing reversible crystallization over a reproducible and well-defined temperature range (e.g., the copolymer exhibits a melting and freezing point as determined, for example, by differential scanning calorimetry).

Preferred PCC's are monomers whose homopolymeric analogs are respectively capable of independently and reversibly crystallizing at or above room temperature (22° C.). Advantageously preferred liquid toner particles according to the invention provide lower fusing temperatures, as compared to otherwise identical liquid toner particles that lack the PCC chemically incorporated into the amphipathic copolymer. Without intending to be bound by a particular theory, it is believed that once the portions of the copolymer containing crystalline material have melted, these portions help to lower the apparent  $T_g$  of the copolymer, thereby providing toner particles that exhibit lower fusing temperatures.

For example, in preferred embodiments where one or more PCC's are incorporated into the D portion of the amphipathic copolymer, the toner particles can fuse at temperatures of about 140–175° C., as compared to fusing temperatures of about 200–250° C. that are observed with otherwise identical toner particles that lack the PCC in the copolymer. During fusing, the portion of the copolymer containing crystalline material melts and the copolymer begins to soften or flow at temperatures just above the melting point of the crystalline material derived from the PCC. After fusing, the portion of the copolymer containing crystalline material solidifies, and excellent blocking resistance is observed at temperatures up to about the melting temperature ( $T_m$ ) of the crystalline material derived from the PCC. Consequently, lower fusing temperatures may be used to obtain fused prints that have excellent durability, particularly with respect to erasure resistance. As a result, printing equipment used in conjunction with preferred liquid toner

particles of the invention do not require as much energy to fuse toner particles onto the final substrate.

In some preferred embodiments, the PCC is incorporated in the D portion of the amphipathic copolymer. According to these embodiments, the PCC is not as readily exposed to and solvatable in the liquid carrier as the S portion. Surprisingly, the lower fusing temperature characteristic of the present invention is observed even when the crystalline material is located in the D portion.

Inclusion of PCC's in the D portion of the amphipathic copolymer provides a liquid toner particle that exhibits improved resistance against blocking (reduced tackiness), as compared to otherwise identical liquid toners that lack the crystalline material in the copolymer. In some preferred embodiments, PCC's include monomers whose homopolymeric analogs are respectively capable of independently and reversibly crystallizing in the range of about 38° C. to 63° C. According to these preferred embodiments of the invention, improved blocking resistance will tend to be observed at temperatures above room temperature but below the crystallization temperature of the PCC derived material.

In addition, inclusion of PCC's in the D and/or S portion of the copolymer can, in some embodiments, eliminate the need to use slip agents, waxes, fuser oils or low surface energy fuser surfaces to prevent or reduce fuser offset. This can provide for fewer ingredients or fewer processing steps in the toner manufacturing process, eliminate the likelihood of surface contamination by non-chemically bonded waxes or fuser oils as used with conventional dry toners, permit use of conventional fuser roller materials over a wider temperature range, and reduced cost associated with fabricating the organosol-derived dry toner or the low temperature fusing system of the electrophotographic printing device.

When the PCC's are incorporated in the D portion of the amphipathic copolymer, it is surprising that the anti-blocking effect is observed, since this portion of the copolymer is not a crystallizable side chain and is therefore not as readily exposed to and solvated in the liquid carrier as the S portion of the copolymer. Further, it is unexpected that the S portion of the copolymer does not interfere with the anti-blocking benefit observed in the inventive toner particles. Further, with respect to embodiments wherein the PCC's are incorporated in the D portion, it is surprising that these PCC's can be included in the D portion without adversely affecting properties of the amphipathic copolymer. The PCC's described herein tend to be soluble in nonaqueous liquid carriers; thus, inclusion of a soluble component in the otherwise dispersed D portion may be expected to adversely impact solubility characteristics of the copolymer, particularly by increasing solubility of the D portion to the point where a relatively high viscosity solution polymer, rather than a relatively low viscosity dispersion polymer (organosol), is obtained.

Moreover, placement of the PCC's in the D portion of the copolymer provides more flexibility in formulating the amphipathic copolymer. As described herein, preferred embodiments of the invention comprise an amphipathic copolymer having a relatively larger amount of D material than S material. By including PCC's in the more abundant D material, greater flexibility is provided in formulating the S material of the copolymer.

Previously, it has been taught that organosols with core (dispersed portion)  $T_g$ 's above room temperature (22° C.) typically do not form cohesive films resulting in poor image transfer in offset printing. It was taught that the integrity of the toned image during partial removal of the solvent also depended upon the core  $T_g$ , with lower  $T_g$  promoting film

strength and image integrity at the cost of additional image tack. See U.S. Pat. No. 6,103,781 (column 11, lines 18–23). Thus, the U.S. Pat. No. 6,103,781 patent describes that preferably, the minimum film forming temperatures are between about 22° C. and 45° C. and the organosol core  $T_g$  is below room temperature to allow the toner to form a film and maintain good image integrity during solvent removal and good cohesive strength during image transfer from the photoconductor onto either a transfer medium or receptor. (U.S. Pat. No. 6,103,781, column 11, lines 23–31).

However, it has been surprisingly found that providing a PCC in the insoluble D portion of the copolymeric constituent of the organosol provides excellent image quality, with reduced tack after fusing to the final image receptor. In some preferred embodiments, incorporation of the PCC in the D portion of the copolymer is effective in promoting rapid self-fixing of the toners in the liquid electrophotographic imaging process even when the calculated  $T_g$  of the D portion is above room temperature (22° C.). In other words, inclusion of a PCC in copolymeric binder having a D portion  $T_g$  above room temperature provides surprising benefits with respect to image quality and image defect elimination, as described herein. Incorporation of a PCC in the D portion of a low  $T_g$  ( $T_g < 22^\circ\text{C}$ .) copolymer is effective at permitting more rapid rates of image self-fixing or film formation in a liquid electrophotographic imaging process, while still serving to reduce toned image tack and improve durability (e.g. blocking and erasure resistance) after fusing to the final image receptor.

In one aspect, the invention provides a liquid electrophotographic toner composition comprising a liquid carrier having a Kauri-Butanol number less than 30, and a plurality of toner particles dispersed in the liquid carrier, wherein the toner particles comprise at least one amphipathic copolymer comprising one or more S material portions and one or more D material portions, wherein one or more of the D material portions chemically comprises one or more polymerizable, crystallizable compounds.

In another aspect, the invention provides a liquid electrophotographic toner composition comprising a liquid carrier having a Kauri-Butanol number less than 30, and a plurality of toner particles dispersed in the liquid carrier, wherein the toner particles comprise at least one amphipathic copolymer, wherein the D portion of the copolymer has a high glass transition temperature ( $T_g$ , above about 55° C.) and at least one polymerizable, crystallizable compound is chemically incorporated into the D portion, the S portion, or both the D portion and S portion of the copolymer. In another aspect, the invention provides a liquid electrophotographic toner composition comprising a liquid carrier having a Kauri-Butanol number less than 30, and a plurality of toner particles dispersed in the liquid carrier, wherein the toner particles comprise at least one amphipathic copolymer, wherein the D portion of the copolymer has a glass transition temperature in the range of about 30° C. to about 50° C., and at least one polymerizable, crystallizable compound is chemically incorporated into the D portion, the S portion, or both the D portion and S portion of the copolymer.

In another aspect, the invention provides a method of making a liquid electrographic toner composition comprising steps of providing an organosol comprising a plurality of toner particles dispersed in a liquid carrier, wherein the toner particles comprise at least one amphipathic copolymer, wherein the amphipathic copolymer comprises one or more S material portions and one or more D material portions, and wherein one or more of the D material portions is chemically incorporated into one or more polymerizable, crystallizable

compounds, and mixing the organosol with one or more additives under conditions effective to form a dispersion. The toner is particularly useful for liquid electrophotographic printing applications.

In another aspect, the invention provides a method of making a liquid electrographic toner composition comprising steps of providing an organosol comprising a plurality of toner particles dispersed in a liquid carrier, wherein the toner particles comprise at least one amphipathic copolymer including a dispersed (D) portion and a solvated (S) portion; and wherein the D portion has a high glass transition temperature ( $T_g$  above about 55° C.) and at least one polymerizable, crystallizable compound is chemically incorporated into the D portion, the S portion, or both the D portion and S portion of the copolymer; and mixing the organosol with one or more additives under conditions effective to form a dispersion. The toner is particularly useful for liquid electrophotographic printing applications.

In another aspect, the invention provides a method of electrophotographically forming an image on a substrate surface comprising steps of providing a liquid toner composition, the liquid toner composition comprising an organosol, wherein the organosol comprises a plurality of toner particles dispersed in a liquid carrier, wherein the toner particles comprise at least one amphipathic copolymer comprising one or more S material portions and one or more D material portions, wherein one or more of the D material portions comprise one or more polymerizable, crystallizable compounds; and causing an image comprising the toner particles to be formed on the substrate surface.

In yet another aspect, the invention provides a method of electrophotographically forming an image on a final image receptor surface comprising steps of:

- (a) providing a liquid toner composition, the liquid toner composition comprising an organosol comprising a plurality of toner particles dispersed in a liquid carrier, wherein the toner particles comprise at least one amphipathic copolymer comprising one or more S material portions and one or more D material portions; and wherein at least one of the D material portions comprises one or more polymerizable, crystallizable compounds;
- (b) causing an image comprising the toner composition to be formed on a charged surface; and
- (c) transferring the image from the charged surface to the final image receptor surface.

In still another aspect the invention provides a method of electrophotographically forming an image on a final image receptor surface comprising steps of:

- (a) providing a liquid toner composition; the liquid toner composition comprising a plurality of toner particles dispersed in a liquid carrier, wherein the toner particles incorporate an organosol comprising at least one amphipathic copolymer including a dispersed (D) portion and a solvated (S) portion; and wherein the D portion has a high glass transition temperature ( $T_g$  above about 55° C.); and at least one polymerizable, crystallizable compound is chemically incorporated into the D portion, the S portion, or both the D portion and S portion of the copolymer
- (b) causing an image comprising the toner composition to be fanned on a charged photoreceptor surface; and
- (c) transferring the image from the charged photoreceptor surface to the final image receptor surface without film formation of the raced image on the photoreceptor.

These and other aspects of the invention will now be described in more detail.

## 11

DETAILED DESCRIPTION OF PRESENTLY  
PREFERRED EMBODIMENTS

The embodiments of the present invention described below are not intended to be exhaustive or to limit the invention to the precise forms disclosed in the following detailed description. Rather, the embodiments are chosen and described so that others skilled in the art can appreciate and understand the principles and practices of the present invention.

Preferably, the nonaqueous liquid carrier of the organosol is selected such that at least one portion (also referred to herein as the S material or portion) of the amphipathic copolymer is more solvated by the carrier while at least one other portion (also referred to herein as the D material or portion) of the copolymer constitutes more of a dispersed phase in the carrier. In other words, preferred copolymers of the present invention comprise S and D material having respective solubilities in the desired liquid carrier that are sufficiently different from each other such that the S blocks tend to be more solvated by the carrier while the D blocks tend to be more dispersed in the carrier. More preferably, the S blocks are soluble in the liquid carrier while the D blocks are insoluble. In particularly preferred embodiments, the D material phase separates from the liquid carrier, forming dispersed particles.

From one perspective, the polymer particles when dispersed in the liquid carrier may be viewed as having a core/shell structure in which the D material tends to be in the core, while the S material tends to be in the shell. The S material thus functions as a dispersing aid, steric stabilizer or graft copolymer stabilizer, to help stabilize dispersions of the copolymer particles in the liquid carrier. Consequently, the S material may also be referred to herein as a "graft stabilizer." The core/shell structure of the binder particles tends to be retained when the particles are dried when incorporated into liquid toner compositions.

The solubility of a material, or a portion of a material such as a copolymeric portion, may be qualitatively and quantitatively characterized in terms of its Hildebrand solubility parameter. The Hildebrand solubility parameter refers to a solubility parameter represented by the square root of the cohesive energy density of a material, having units of  $(\text{pressure})^{1/2}$ , and being equal to  $(\Delta H/RT)^{1/2}/V^{1/2}$ , where  $\Delta H$  is the molar vaporization enthalpy of the material,  $R$  is the universal gas constant,  $T$  is the absolute temperature, and  $V$  is the molar volume of the solvent. Hildebrand solubility parameters are tabulated for solvents in Barton, A. F. M., *Handbook of Solubility and Other Cohesion Parameters*, 2d Ed. CRC Press, Boca Raton, Fla., (1991), for monomers and representative polymers in *Polymer Handbook*, 3rd Ed., J. Brandrup & E. H. Immergut, Eds. John Wiley, N.Y., pp 519-557 (1989), and for many commercially available polymers in Barton, A. F. M., *Handbook of Polymer-Liquid Interaction Parameters and Solubility Parameters*, CRC Press, Boca Raton, Fla., (1990).

The degree of solubility of a material, or portion thereof, in a liquid carrier may be predicted from the absolute difference in Hildebrand solubility parameters between the material, or portion thereof, and the liquid carrier. A material, or portion thereof, will be fully soluble or at least in a highly solvated state when the absolute difference in Hildebrand solubility parameter between the material, or portion thereof, and the liquid carrier is less than approximately  $1.5 \text{ MPa}^{1/2}$ . On the other hand, when the absolute difference between the Hildebrand solubility parameters exceeds approximately  $3.0 \text{ MPa}^{1/2}$ , the material, or portion thereof,

## 12

will tend to phase separate from the liquid carrier, forming a dispersion. When the absolute difference in Hildebrand solubility parameters is between  $1.5 \text{ MPa}^{1/2}$  and  $3.0 \text{ MPa}^{1/2}$ , the material, or portion thereof, is considered to be weakly solvatable or marginally insoluble in the liquid carrier.

Consequently, in preferred embodiments, the absolute difference between the respective Hildebrand solubility parameters of the S portion(s) of the copolymer and the liquid carrier is less than  $3.0 \text{ MPa}^{1/2}$ , preferably less than about  $2.0 \text{ MPa}^{1/2}$ , more preferably less than about  $1.5 \text{ MPa}^{1/2}$ . In a particularly preferred embodiment of the present invention, the absolute difference between the respective Hildebrand solubility parameters of the S portion(s) of the copolymer and the liquid carrier is from about 2 to about  $3.0 \text{ MPa}^{1/2}$ . Additionally, it is also preferred that the absolute difference between the respective Hildebrand solubility parameters of the D portion(s) of the copolymer and the liquid carrier is greater than  $2.3 \text{ MPa}^{1/2}$ , preferably greater than about  $2.5 \text{ MPa}^{1/2}$ , more preferably greater than about  $3.0 \text{ MPa}^{1/2}$ , with the proviso that the difference between the respective Hildebrand solubility parameters of the S and D portion(s) is at least about  $0.4 \text{ MPa}^{1/2}$ , more preferably at least about  $1.0 \text{ MPa}^{1/2}$ . Because the Hildebrand solubility of a material may vary with changes in temperature, such solubility parameters are preferably determined at a desired reference temperature such as at  $25^\circ \text{C}$ .

Those skilled in the art understand that the Hildebrand solubility parameter for a copolymer, or portion thereof, may be calculated using a volume fraction weighting of the individual Hildebrand solubility parameters for each monomer comprising the copolymer, or portion thereof, as described for binary copolymers in Barton A. F. M., *Handbook of Solubility Parameters and Other Cohesion Parameters*, CRC Press, Boca Raton, p 12 (1990). The magnitude of the Hildebrand solubility parameter for polymeric materials is also known to be weakly dependent upon the weight average molecular weight of the polymer, as noted in Barton, pp 446-448. Thus, there will be a preferred molecular weight range for a given polymer or portion thereof in order to achieve desired solvating or dispersing characteristics. Similarly, the Hildebrand solubility parameter for a mixture may be calculated using a volume fraction weighting of the individual Hildebrand solubility parameters for each component of the mixture.

In addition, we have defined our invention in terms of the calculated solubility parameters of the monomers and solvents obtained using the group contribution method developed by Small, P. A., *J. Appl. Chem.*, 3, 71 (1953) using Small's group contribution values listed in Table 2.2 on page VII/525 in the *Polymer Handbook*, 3rd Ed., J. Brandrup & E. H. Immergut, Eds. John Wiley, New York, (1989). We have chosen this method for defining our invention to avoid ambiguities that could result from using solubility parameter values obtained with different experimental methods. In addition, Small's group contribution values will generate solubility parameters that are consistent with data derived from measurements of the enthalpy of vaporization, and therefore are completely consistent with the defining expression for the Hildebrand solubility parameter. Since it is not practical to measure the heat of vaporization for polymers, monomers are a reasonable substitution.

For purposes of illustration, Table I lists Hildebrand solubility parameters for some common solvents used in an electrophotographic toner and the Hildebrand solubility parameters and glass transition temperatures (based on their

## 13

high molecular weight homopolymers) for some common monomers used in synthesizing organosols.

TABLE I

| Hildebrand Solubility Parameters |                                                    |                                                       |
|----------------------------------|----------------------------------------------------|-------------------------------------------------------|
| Solvent Values at 25° C.         |                                                    |                                                       |
| Solvent Name                     | Kauri-Butanol Number by ASTM Method D1133-54T (ml) | Hildebrand Solubility Parameter (MPa <sup>1/2</sup> ) |
| Norpar™ 15                       | 18                                                 | 13.99                                                 |
| Norpar™ 13                       | 22                                                 | 14.24                                                 |
| Norpar™ 12                       | 23                                                 | 14.30                                                 |
| Isopar™ V                        | 25                                                 | 14.42                                                 |
| Isopar™ G                        | 28                                                 | 14.60                                                 |
| Exxsol™ D80                      | 28                                                 | 14.60                                                 |

Source: Calculated from equation #31 of Polymer Handbook, 3<sup>rd</sup> Ed., J. Brandrup E. H. Immergut, Eds. John Wiley, NY, p. VII/522 (1989).

## Monomer Values at 25° C.

| Monomer Name                            | Hildebrand Solubility Parameter (MPa <sup>1/2</sup> ) | Glass Transition Temperature (° C.)* |
|-----------------------------------------|-------------------------------------------------------|--------------------------------------|
| 3,3,5-Trimethyl Cyclohexyl Methacrylate | 16.73                                                 | 125                                  |
| Isobornyl Methacrylate                  | 16.90                                                 | 110                                  |
| Isobornyl Acrylate                      | 16.01                                                 | 94                                   |
| n-Behenyl Acrylate                      | 16.74                                                 | <55 (58 m.p.)**                      |
| n-Octadecyl Methacrylate                | 16.77                                                 | -100 (45 m.p.)**                     |
| n-Octadecyl Acrylate                    | 16.82                                                 | -55                                  |
| Lauryl Methacrylate                     | 16.84                                                 | -65                                  |
| Lauryl Acrylate                         | 16.95                                                 | -30                                  |
| 2-Ethylhexyl Methacrylate               | 16.97                                                 | -10                                  |
| 2-Ethylhexyl Acrylate                   | 17.03                                                 | -55                                  |
| n-Hexyl Methacrylate                    | 17.13                                                 | -5                                   |
| t-Butyl Methacrylate                    | 17.16                                                 | 107                                  |
| n-Butyl Methacrylate                    | 17.22                                                 | 20                                   |
| n-Hexyl Acrylate                        | 17.30                                                 | -60                                  |
| n-Butyl Acrylate                        | 17.45                                                 | -55                                  |
| Ethyl Methacrylate                      | 17.62                                                 | 65                                   |
| Ethyl Acrylate                          | 18.04                                                 | -24                                  |
| Methyl Methacrylate                     | 18.17                                                 | 105                                  |
| Styrene                                 | 18.05                                                 | 100                                  |

Calculated using Small's Group Contribution Method, Small, P. A. Journal of Applied Chemistry 3 p. 71 (1953). Using Group Contributions from Polymer Handbook, 3<sup>rd</sup> Ed., J. Brandrup E. H. Immergut, Eds., John Wiley, NY, p. VII/525 (1989).

\*Polymer Handbook, 3<sup>rd</sup> Ed., J. Brandrup E. H. Immergut, Eds., John Wiley, NY, pp. VII/209-277 (1989). The T<sub>g</sub> listed is for the homopolymer of the respective monomer.

\*\*m.p. refers to melting point for selected Polymerizable Crystallizable Compounds.

The liquid carrier is a substantially nonaqueous solvent or solvent blend. In other words, only a minor component (generally less than 25 weight percent) of the liquid carrier comprises water. Preferably, the substantially nonaqueous liquid carrier comprises less than 20 weight percent water, more preferably less than 10 weight percent water, even more preferably less than 3 weight percent water, most preferably less than one weight percent water.

The substantially nonaqueous carrier liquid may be selected from a wide variety of materials, or combination of materials, which are known in the art, but preferably has a Kauri-butanol number less than 30 ml. The liquid is preferably oleophilic, chemically stable under a variety of conditions, and electrically insulating. Electrically insulating refers to a dispersant liquid having a low dielectric constant and a high electrical resistivity. Preferably, the liquid dispersant has a dielectric constant of less than 5; more preferably less than 3. Electrical resistivities of carrier liquids

## 14

are typically greater than 10<sup>9</sup> Ohm-cm, more preferably greater than 10<sup>10</sup> Ohm-cm. In addition, the liquid carrier desirably is chemically inert in most embodiments with respect to the ingredients used to formulate the toner particles.

Examples of suitable liquid carriers include aliphatic hydrocarbons (n-pentane, hexane, heptane and the like), cycloaliphatic hydrocarbons (cyclopentane, cyclohexane and the like), aromatic hydrocarbons (benzene, toluene, xylene and the like), halogenated hydrocarbon solvents (chlorinated alkanes, fluorinated alkanes, chlorofluorocarbons and the like) silicone oils and blends of these solvents. Preferred carrier liquids include branched paraffinic solvent blends such as Isopar™ G, Isopar™ H, Isopar™ K, Isopar™ L, Isopar™ M and Isopar™ V (available from Exxon Corporation, NJ), and most preferred carriers are the aliphatic hydrocarbon solvent blends such as Norpar™ 12, Norpar™ 13 and Norpar™ 15 (available from Exxon Corporation, NJ). Particularly preferred carrier liquids have a Hildebrand solubility parameter of from about 13 to about 15 MPa<sup>1/2</sup>.

As used herein, the term "copolymer" encompasses both oligomeric and polymeric materials, and encompasses polymers incorporating two or more monomers. As used herein, the term "monomer" means a relatively low molecular weight material (i.e., generally having a molecular weight less than about 500 Daltons) having one or more polymerizable groups. "Oligomer" means a relatively intermediate sized molecule incorporating two or more monomers and generally having a molecular weight of from about 500 up to about 10,000 Daltons. "Polymer" means a relatively large material comprising a substructure formed two or more monomeric, oligomeric, and/or polymeric constituents and generally having a molecular weight greater than about 10,000 Daltons.

The term "macromer" or "macromonomer" refers to an oligomer or polymer having a terminal polymerizable moiety. "Polymerizable crystallizable compound" or "PCC" refers to compounds capable of undergoing polymerization to produce a copolymer wherein at least a portion of the copolymer is capable of undergoing reversible crystallization over a reproducible and well-defined temperature range (e.g. the copolymer exhibits a melting and freezing point as determined, for example, by differential scanning calorimetry). PCC's may include monomers, functional oligomers, functional pre-polymers, macromers or other compounds able to undergo polymerization to form a copolymer. The term "molecular weight" as used throughout this specification means weight average molecular weight unless expressly noted otherwise.

The weight average molecular weight of the amphipathic copolymer of the present invention may vary over a wide range, and may impact imaging performance. The polydispersity of the copolymer also may impact imaging and transfer performance of the resultant toner composition. Because of the difficulty of measuring molecular weight for an amphipathic copolymer, the particle size of the dispersed copolymer (organosol) may instead be correlated to imaging and transfer performance of the resultant toner composition. Generally, the volume mean particle diameter (D<sub>v</sub>) of the dispersed graft copolymer particles, determined by laser diffraction particle size measurement, should be in the range 0.1-100 microns, more preferably 0.5-50 microns, even more preferably 1.0-20 microns, and most preferably 2-10 microns.

In addition, a correlation exists between the molecular weight of the solvatable or soluble S portion of the graft

copolymer, and the imaging and transfer performance of the resultant toner. Generally, the S portion of the copolymer has a weight average molecular weight in the range of 1000 to about 1,000,000 Daltons, preferably 5000 to 400,000 Daltons, more preferably 50,000 to 300,000 Daltons. It is also generally desirable to maintain the polydispersity (the ratio of the weight-average molecular weight to the number average molecular weight) of the S portion of the copolymer below 15, more preferably below 5, most preferably below 2.5. It is a distinct advantage of the present invention that copolymer particles with such lower polydispersity characteristics for the S portion are easily made in accordance with the practices described herein, particularly those embodiments in which the copolymer is formed in the liquid carrier *in situ*.

The relative amounts of S and D portions in a copolymer can impact the solvating and dispersability characteristics of these portions. For instance, if too little of the S portion(s) are present, the copolymer may have too little stabilizing effect to sterically-stabilize the organosol with respect to aggregation as might be desired. If too little of the D portion(s) are present, the small amount of D material may be too soluble in the liquid carrier such that there may be insufficient driving force to form a distinct particulate, dispersed phase in the liquid carrier. The presence of both a solvated and dispersed phase helps the ingredients of particles self assemble *in situ* with exceptional uniformity among separate particles. Balancing these concerns, the preferred weight ratio of D material to S material is in the range of 1:20 to 20:1, preferably 1:1 to 15:1, more preferably 2:1 to 10:1, and most preferably 4:1 to 8:1.

Glass transition temperature,  $T_g$ , refers to the temperature at which a (co)polymer, or portion thereof, changes from a hard, glassy material to a rubbery, or viscous, material, corresponding to a dramatic increase in free volume as the (co)polymer is heated. The  $T_g$  can be calculated for a (co)polymer, or portion thereof, using known  $T_g$  values for the high molecular weight homopolymers (see, e.g., Table I herein) and the Fox equation expressed below:

$$1/T_g = w_1/T_{g1} + w_2/T_{g2} + \dots + w_r/T_{gr}$$

wherein each  $w_n$  is the weight fraction of monomer "n" and each  $T_{gn}$  is the absolute glass transition temperature (in degrees Kelvin) of the high molecular weight homopolymer of monomer "n" as described in Wicks, A. W., F. N. Jones & S. P. Pappas, *Organic Coatings 1*, John Wiley, NY, pp 54-55 (1992).

In the practice of the present invention, values of  $T_g$  for the D or S portion of the copolymer were determined using the Fox equation above, although the  $T_g$  of the copolymer as a whole may be determined experimentally using e.g. differential scanning calorimetry. The glass transition temperatures ( $T_g$ 's) of the S and D portions may vary over a wide range and may be independently selected to enhance manufacturability and/or performance of the resulting toner compositions. The  $T_g$ 's of the S and D portions will depend to a large degree upon the type of monomers constituting such portions. Consequently, to provide a copolymer material with higher  $T_g$ , one can select one or more higher  $T_g$  monomers with the appropriate solubility characteristics for the type of copolymer portion (D or S) in which the monomer(s) will be used. Conversely, to provide a copolymer material with lower  $T_g$ , one can select one or more lower  $T_g$  monomers with the appropriate solubility characteristics for the type of portion in which the monomer(s) will be used.

For copolymers useful in liquid toner applications, the copolymer  $T_g$  preferably should not be too low or else receptors printed with the toner may experience undue blocking. Conversely, the minimum fusing temperature required to soften or melt the toner particles sufficient for them to adhere to the final image receptor will increase as the copolymer  $T_g$  increases. Consequently, it is preferred that the  $T_g$  of the copolymer be far enough above the expected maximum storage temperature of a printed receptor so as to avoid blocking issues, yet not so high as to require fusing temperatures approaching the temperatures at which the final image receptor may be damaged, e.g. approaching the autoignition temperature of paper used as the final image receptor. In this regard, incorporation of a polymerizable crystallizable compound (PCC) in the copolymer will generally permit use of a lower copolymer  $T_g$  and therefore lower fusing temperatures without the risk of the image blocking at storage temperatures below the melting temperature of the PCC. Desirably, therefore, the copolymer has a  $T_g$  of 0°-100° C., more preferably 20°-80° C., most preferably 40°-70° C.

For copolymers in which the D portion comprises a major portion of the copolymer, the  $T_g$  of the D portion will dominate the  $T_g$  of the copolymer as a whole. For such copolymers useful in liquid toner applications, it is preferred that the  $T_g$  of the D portion fall in the range of 20°-105° C., more preferably 30°-85° C., most preferably 60°-75° C., since the S portion will generally exhibit a lower  $T_g$  than the D portion, and a higher  $T_g$  D portion is therefore desirable to offset the  $T_g$  lowering effect of the S portion, which may be solvatable. In this regard, incorporation of a polymerizable crystallizable compound (PCC) in the D portion of the copolymer will generally permit use of a lower D portion  $T_g$  and therefore lower fusing temperatures without the risk of the image blocking at storage temperatures below the melting temperature of the PCC.

Blocking with respect to the S portion material is not as significant an issue inasmuch as preferred copolymers comprise a majority of the D portion material. Consequently, the  $T_g$  of the D portion material will dominate the effective  $T_g$  of the copolymer as a whole. However, if the  $T_g$  of the S portion is too low, then the particles might tend to aggregate. On the other hand, if the  $T_g$  is too high, then the requisite fusing temperature may be too high. Balancing these concerns, the S portion material is preferably formulated to have a  $T_g$  of at least 0° C., preferably at least 20° C., more preferably at least 40° C. In this regard, incorporation of a polymerizable crystallizable compound (PCC) in the S portion of the copolymer will generally permit use of a lower S portion  $T_g$ .

It is understood that the requirements imposed on the self-fixing characteristics of a liquid toner will depend to a great extent upon the nature of the imaging process. For example, rapid self-fixing of the toner to form a cohesive film may not be required or even desired in an electrographic imaging process if the image is not subsequently transferred to a final receptor, or if the transfer is effected by means (e.g. electrostatic transfer) not requiring a film formed toner on a temporary image receptor (e.g. a photoreceptor). Similarly, in multi-color (or multi-pass) electrostatic printing wherein a stylus is used to generate a latent electrostatic image directly upon a dielectric receptor that serves as the final toner receptor material, a rapidly self-fixing toner film may be undesirably removed in passing under the stylus. This head scraping can be reduced or eliminated by manipulating the effective glass transition temperature of the organosol. For liquid electrographic (electrostatic) toners, particularly

liquid toners developed for use in direct electrostatic printing processes, the D portion of the organosol is preferably provided with a sufficiently high  $T_g$  such that the organosol exhibits an effective glass transition temperature of from about 15° C. to about 55° C., and the D portion exhibits a  $T_g$  calculated using the Fox equation, of about 30–55° C. Liquid toners having both a polymerizable crystalline compound in the organosol and having an effective glass transition temperature of about 15–55° C. provide particular benefit in the multipass electrostatic printing process as described above, because the toner exhibits both excellent fusing temperature and superior resistance to marring or scraping either during or after the image is printed. A wide variety of one or more different monomeric, oligomeric and/or polymeric materials may be independently incorporated into the S and D portions, as desired. Representative examples of suitable materials include free radically polymerized material (also referred to as vinyl copolymers or (meth) acrylic copolymers in some embodiments), polyurethanes, polyester, epoxy, polyamide, polyimide, polysiloxane, fluoropolymer, polysulfone, combinations of these, and the like. Preferred S and D portions are derived from free radically polymerizable material. In the practice of the present invention, "free radically polymerizable" refers to monomers, oligomers, and/or polymers having functionality directly or indirectly pendant from a monomer, oligomer, or polymer backbone (as the case may be) that participate in polymerization reactions via a free radical mechanism. Representative examples of such functionality includes (meth) acrylate groups, olefinic carbon-carbon double bonds, allyloxy groups, alpha-methyl styrene groups, (meth)acrylamide groups, cyanate ester groups, vinyl ether groups, combinations of these, and the like. The term "(meth)acryl", as used herein, encompasses acryl and/or methacryl.

Free radically polymerizable monomers, oligomers, and/or polymers are advantageously used to form the copolymer in that so many different types are commercially available and may be selected with a wide variety of desired characteristics that help provide one or more desired performance characteristics. Free radically polymerizable monomers, oligomers, and/or monomers suitable in the practice of the present invention may include one or more free radically polymerizable moieties.

Representative examples of monofunctional, free radically polymerizable monomers include styrene, alpha-methylstyrene, substituted styrene, vinyl esters, vinyl ethers, N-vinyl-2-pyrrolidone, (meth)acrylamide, vinyl naphthalene, alkylated vinyl naphthalenes, alkoxy vinyl naphthalenes, N-substituted (meth)acrylamide, octyl (meth)acrylate, nonylphenol ethoxylate (meth)acrylate, N-vinyl pyrrolidone, isononyl (meth)acrylate, isobornyl (meth)acrylate, 2-(2-ethoxyethoxy)ethyl (meth)acrylate, 2-ethylhexyl (meth)acrylate, beta-carboxyethyl (meth)acrylate, isobutyl (meth)acrylate, cycloaliphatic epoxide, alpha-epoxide, 2-hydroxyethyl (meth)acrylate, (meth)acrylonitrile, maleic anhydride, itaconic acid, isodecyl (meth)acrylate, lauryl (dodecyl) (meth)acrylate, stearyl (octadecyl) (meth)acrylate, behenyl (meth)acrylate, n-butyl(meth)acrylate, methyl (meth)acrylate, ethyl (meth)acrylate, hexyl (meth)acrylate, (meth)acrylic acid, N-vinylcaprolactam, stearyl (meth)acrylate, hydroxy functional caprolactone ester (meth)acrylate, isoctyl (meth)acrylate, hydroxyethyl (meth)acrylate, hydroxymethyl (meth)acrylate, hydroxypropyl (meth)acrylate, hydroxyisopropyl (meth)acrylate, hydroxybutyl (meth)acrylate, hydroxyisobutyl (meth)acrylate, tetrahydrofurfuryl (meth)acrylate, isobornyl (meth)acrylate, glycidyl (meth)acrylate vinyl acetate, combinations of these, and the like.

Preferred copolymers of the present invention may be formulated with one or more radiation curable monomers or combinations thereof that help the free radically polymerizable compositions and/or resultant cured compositions to satisfy one or more desirable performance criteria. For example, in order to promote hardness and abrasion resistance, a formulator may incorporate one or more free radically polymerizable monomer(s) (hereinafter "high  $T_g$  component") whose presence causes the polymerized material, or a portion thereof, to have a higher glass transition temperature,  $T_g$ , as compared to an otherwise identical material lacking such high  $T_g$  component. Preferred monomeric constituents of the high  $T_g$  component generally include monomers whose homopolymers have a  $T_g$  of at least about 50° C., preferably at least about 60° C., and more preferably at least about 75° C. in the cured state.

An exemplary class of radiation curable monomers that tend to have relatively high  $T_g$  characteristics suitable for incorporation into the high  $T_g$  component generally comprises at least one radiation curable (meth)acrylate moiety and at least one nonaromatic, alicyclic and/or nonaromatic heterocyclic moiety. Isobornyl (meth)acrylate is a specific example of one such monomer. A cured, homopolymer film formed from isobornyl acrylate, for instance, has a  $T_g$  of 110° C. The monomer itself has a molecular weight of 222 g/mole, exists as a clear liquid at room temperature, has a viscosity of 9 centipoise at 25° C., and has a surface tension of 31.7 dynes/cm at 25° C. Additionally, 1,6-Hexanediol di(meth)acrylate is another example of a monomer with high  $T_g$  characteristics.

Trimethyl cyclohexyl methacrylate (TCHMA) is another example of a high  $T_g$  monomer useful in the practice of the present invention. TCHMA has a  $T_g$  of 125° C. and tends to be solvatable in oleophilic solvents. Consequently, TCHMA is easily incorporated into S material. However, if used in limited amounts so as not to unduly impair the insolubility characteristics of D material, some TCHMA may also be incorporated into the D material.

The advantages of incorporating high  $T_g$  monomers into the copolymer are further described in assignee's co-pending U.S. patent application Ser. No. 10/612,765 titled ORGANOSOL INCLUDING HIGH  $T_g$  AMPHIPATHIC COPOLYMERIC BINDER AND LIQUID TONERS FOR ELECTROPHOTOGRAPHIC APPLICATIONS and filed on the same day as the present application in the names of Julie Y. Qian et al. The advantages of incorporating soluble high  $T_g$  monomer into the copolymer are further described in assignee's co-pending U.S. patent application Ser. No. 10/612,533 titled ORGANOSOL INCLUDING AMPHIPATHIC COPOLYMERIC BINDER MADE WITH SOLUBLE HIGH  $T_g$  MONOMER AND LIQUID TONERS FOR ELECTROPHOTOGRAPHIC APPLICATIONS and filed on the same day as the present application in the names of Julie Y. Qian et al. Both of these co-pending patent applications are hereby incorporated herein by reference in their entirety.

Nitrile functionality may be advantageously incorporated into the copolymer for a variety of reasons, including improved durability, enhanced compatibility with visual enhancement additive(s), e.g., colorant particles, and the like. In order to provide a copolymer having pendant nitrile groups, one or more nitrile functional monomers can be used. Representative examples of such monomers include (meth)acrylonitrile,  $\beta$ -cyanoethyl-(meth)acrylate, 2-cyanoethoxyethyl (meth)acrylate, p-cyanostyrene, p-(cyanomethyl)styrene, N-vinylpyrrolidinone, and the like.

In order to provide a copolymer having pendant hydroxyl groups, one or more hydroxyl functional monomers can be used. Pendant hydroxyl groups of the copolymer not only facilitate dispersion and interaction with the pigments in the formulation, but also promote solubility, cure, reactivity with other reactants, and compatibility with other reactants. The hydroxyl groups can be primary, secondary, or tertiary, although primary and secondary hydroxyl groups are preferred. When used, hydroxy functional monomers constitute from about 0.5 to 30, more preferably 1 to about 25 weight percent of the monomers used to formulate the copolymer, subject to preferred weight ranges for graft copolymers noted below.

Representative examples of suitable hydroxyl functional monomers include an ester of an  $\alpha$ ,  $\beta$ -unsaturated carboxylic acid with a diol, e.g., 2-hydroxyethyl (meth)acrylate, or 2-hydroxypropyl (meth)acrylate; 1,3-dihydroxypropyl-2-(meth)acrylate; 2,3-dihydroxypropyl-1-(meth)acrylate; an adduct of an  $\alpha$ ,  $\beta$ -unsaturated carboxylic acid with caprolactone; an alkanol vinyl ether such as 2-hydroxyethyl vinyl ether; 4-vinylbenzyl alcohol; allyl alcohol; p-methylol styrene; or the like.

In certain preferred embodiments, polymerizable crystallizable compounds, e.g. crystalline monomer(s) are chemically incorporated into the copolymer. The term "crystalline monomer" refers to a monomer whose homopolymeric analog is capable of independently and reversibly crystallizing at or above room temperature (e.g., 22° C.).

In these embodiments, the resulting toner particles can exhibit improved blocking resistance between printed receptors and reduced offset during fusing. If used, one or more of these crystalline monomers may be incorporated into the D material of the copolymer. Suitable crystalline monomers include alkyl(meth)acrylates where the alkyl chain contains more than 13 carbon atoms (e.g. tetradecyl(meth)acrylate, pentadecyl(meth)acrylate, hexadecyl(meth)acrylate, heptadecyl(meth)acrylate, octadecyl(meth)acrylate, etc). Other suitable crystalline monomers whose homopolymers have melting points above 22° C. include aryl acrylates and methacrylates; high molecular weight alpha olefins; linear or branched long chain alkyl vinyl ethers or vinyl esters; long chain alkyl isocyanates; unsaturated long chain polyesters, polysiloxanes and polysilanes; polymerizable natural waxes with melting points above 22° C., polymerizable synthetic waxes with melting points above 22° C., and other similar type materials known to those skilled in the art. As described herein, incorporation of crystalline monomers in the copolymer provides surprising benefits to the resulting liquid toner compositions.

Other suitable crystalline monomers include hexacontanyl (meth)acrylate, pentacosanyl (meth)acrylate, behenyl (meth)acrylate, octadecyl (meth)acrylate, hexadecyl acrylate, and tetradecyl acrylate.

It will be understood by those skilled in the art that blocking resistance can be observed at temperatures above room temperature but below the crystallization temperature of the polymer portion incorporating the crystalline monomers or other polymerizable crystallizable compound. Many crystalline monomers tend to be soluble in oleophilic solvents commonly used as liquid carrier material(s) in an organosol. Thus, crystalline material is relatively easily incorporated into S material without impacting desired solubility characteristics. However, if too much of such crystalline material were to be incorporated into D material, the resultant D material may tend to be too soluble in the organosol. Yet, so long as the amount of soluble, crystalline material in the D material is limited, some amount of

crystalline material may be advantageously incorporated into the D material without unduly impacting the desired insolubility characteristics. Thus, when present in the D material, the crystalline material is preferably provided in an amount of up to about 30%, more preferably up to about 20%, most preferably up to about 5% to 10% of the total D material incorporated into the copolymer.

When crystalline monomers or PCC's are chemically incorporated into the D material, suitable co-polymerizable compounds to be used in combination with the PCC include monomers (including other PCC's) such as 2-ethylhexyl acrylate, 2-ethylhexyl (methacrylate), lauryl acrylate, lauryl methacrylate, octadecyl acrylate, octadecyl(methacrylate), isobornyl acrylate, isobornyl (methacrylate), hydroxy(ethyl)methacrylate, and other acrylates and methacrylates.

Multifunctional free radically reactive materials may also be used to enhance one or more properties of the resultant toner particles, including crosslink density, hardness, tackiness, mar resistance, or the like. Examples of such higher functional, monomers include ethylene glycol di(meth)acrylate, hexanediol di(meth)acrylate, triethylene glycol di(meth)acrylate, tetraethylene glycol di(meth)acrylate, trimethylol-propane tri(meth)acrylate, ethoxylated trimethylolpropane tri(meth)acrylate, glycerol tri(meth)acrylate, pentaerythritol tri(meth)acrylate, pentaerythritol tetra(meth)acrylate, and neopentyl glycol di(meth)acrylate, divinyl benzene, combinations of these, and the like.

Suitable free radically reactive oligomer and/or polymeric materials for use in the present invention include, but are not limited to, (meth)acrylated urethanes (i.e., urethane (meth)acrylates), (meth)acrylated epoxies (i.e., epoxy (meth)acrylates), (meth)acrylated polyesters (i.e., polyester (meth)acrylates), (meth)acrylated (meth)acrylics, (meth)acrylated silicones, (meth)acrylated polyethers (i.e., polyether (meth)acrylates), vinyl (meth)acrylates, and (meth)acrylated oils.

Copolymers of the present invention can be prepared by free-radical polymerization methods known in the art, including but not limited to bulk, solution, and dispersion polymerization methods. The resultant copolymers may have a variety of structures including linear, branched, three dimensionally networked, graft-structured, combinations thereof, and the like. A preferred embodiment is a graft copolymer comprising one or more oligomeric and/or polymeric arms attached to an oligomeric or polymeric backbone. In graft copolymer embodiments, the S portion or D portion materials, as the case may be, may be incorporated into the arms and/or the backbone.

Any number of reactions known to those skilled in the art may be used to prepare a free radically polymerized copolymer having a graft structure. Common grafting methods include random grafting of polyfunctional free radicals; copolymerization of monomers with macromonomers; ring-opening polymerizations of cyclic ethers, esters, amides or acetals; epoxidations; reactions of hydroxyl or amino chain transfer agents with terminally-unsaturated end groups; esterification reactions (i.e., glycidyl methacrylate undergoes tertiary-amine catalyzed esterification with methacrylic acid); and condensation polymerization.

Representative methods of forming graft copolymers are described in U.S. Pat. Nos. 6,255,363; 6,136,490; and 5,384,226; and Japanese Published Patent Document No. 05-119529, incorporated herein by reference. Representative examples of grafting methods are also described in sections 3.7 and 3.8 of *Dispersion Polymerization in Organic Media*, K. E. J. Barrett, ed., (John Wiley; New York, 1975) pp. 79-106, also incorporated herein by reference.

Representative examples of grafting methods also may use an anchoring group to facilitate anchoring. The function of the anchoring group is to provide a covalently bonded link between the core part of the copolymer (the D material) and the soluble shell component (the S material). Suitable monomers containing anchoring groups include: adducts of alk-enylazlactone comonomers with an unsaturated nucleophile containing hydroxy, amino, or mercaptan groups, such as 2-hydroxyethylmethacrylate, 3-hydroxypropylmethacrylate, 2-hydroxyethylacrylate, pentaerythritol triacrylate, 4-hydroxybutylvinylether, 9-octadecen-1-ol, cinnamyl alcohol, allyl mercaptan, methylallylamine; and azlactones, such as 2-alkenyl-4,4-dialkylazlactone.

The preferred methodology described above accomplishes grafting via attaching an ethylenically-unsaturated isocyanate (for example, dimethyl-m-isopropenyl benzyl-isocyanate, TMI, available from CYTEC Industries, West Paterson, N.J.; or isocyanatoethyl methacrylate, also known as IEM) to hydroxyl groups in order to provide free radically reactive anchoring groups.

A preferred method of forming a graft copolymer of the present invention involves three reaction steps that are carried out in a suitable substantially nonaqueous liquid carrier in which resultant S material is soluble while D material is dispersed or insoluble.

In a first preferred step, a hydroxyl functional, free radically polymerized oligomer or polymer is formed from one or more monomers, wherein at least one of the monomers has pendant hydroxyl functionality. Preferably, the hydroxyl functional monomer constitutes about 1 to about 30, preferably about 2 to about 10 percent, most preferably 3 to about 5 percent by weight of the monomers used to form the oligomer or polymer of this first step. This first step is preferably carried out via solution polymerization in a substantially nonaqueous solvent in which the monomers and the resultant polymer are soluble. For instance, using the Hildebrand solubility data in Table 1, monomers such as octadecyl methacrylate, octadecyl acrylate, lauryl acrylate, and lauryl methacrylate are suitable for this first reaction step when using an oleophilic solvent such as heptane or the like.

In a second reaction step, all or a portion of the hydroxyl groups of the soluble polymer are catalytically reacted with an ethylenically unsaturated aliphatic isocyanate (e.g. meta-isopropenylidemethylbenzyl isocyanate commonly known as TMI or isocyanatoethyl methacrylate, commonly known as IEM) to form pendant free radically polymerizable functionality that is attached to the oligomer or polymer via a polyurethane linkage. This reaction can be carried out in the same solvent, and hence the same reaction vessel, as the first step. The resultant double-bond functionalized polymer generally remains soluble in the reaction solvent and constitutes the S portion material of the resultant copolymer, which ultimately will constitute at least a portion of the solvatable portion of the resultant triboelectrically charged particles.

The resultant free radically reactive functionality provides grafting sites for attaching D material and optionally additional S material to the polymer. In a third step, these grafting site(s) are used to covalently graft such material to the polymer via reaction with one or more free radically reactive monomers, oligomers, and/or polymers that are initially soluble in the solvent, but then become insoluble as the molecular weight of the graft copolymer. For instance, using the Hildebrand solubility parameters in Table 1, monomers such as e.g. methyl (meth)acrylate, ethyl (meth)acry-

late, t-butyl methacrylate and styrene are suitable for this third reaction step when using an oleophilic solvent such as heptane or the like.

The product of the third reaction step is generally an organosol comprising the resultant copolymer dispersed in the reaction solvent, which constitutes a substantially non-aqueous liquid carrier for the organosol. At this stage, it is believed that the copolymer tends to exist in the liquid carrier as discrete, monodisperse particles having dispersed (e.g., substantially insoluble, phase separated) portion(s) and solvated (e.g., substantially soluble) portion(s). As such, the solvated portion(s) help to sterically-stabilize the dispersion of the particles in the liquid carrier. It can be appreciated that the copolymer is thus advantageously formed in the liquid carrier in situ.

Before further processing, the copolymer particles may remain in the reaction solvent. Alternatively, the particles may be transferred in any suitable way into fresh solvent that is the same or different so long as the copolymer has solvated and dispersed phases in the fresh solvent. In either case, the resulting organosol is then converted into toner particles by mixing the organosol with at least one visual enhancement additive. Optionally, one or more other desired ingredients also can be mixed into the organosol before and/or after combination with the visual enhancement particles. During such combination, it is believed that ingredients comprising the visual enhancement additive and the copolymer will tend to self-assemble into composite particles having a structure wherein the dispersed phase portions generally tend to associate with the visual enhancement additive particles (for example, by physically and/or chemically interacting with the surface of the particles), while the solvated phase portions help promote dispersion in the carrier.

The optional visual enhancement additive(s) generally may include any one or more fluid and/or particulate materials that provide a desired visual effect when toner particles incorporating such materials are printed onto a receptor. Examples include one or more colorants, fluorescent materials, pearlescent materials, iridescent materials, metallic materials, flip-flop pigments, silica, polymeric beads, reflective and non-reflective glass beads, mica, combinations of these, and the like. The amount of visual enhancement additive incorporated into the toner particles may vary over a wide range. In representative embodiments, a suitable weight ratio of copolymer to visual enhancement additive is from 1/1 to 20/1, preferably from 2/1 to 10/1 and most preferably from 4/1 to 8/1.

Useful colorants are well known in the art and include materials listed in the Colour Index, as published by the Society of Dyers and Colourists (Bradford, England), including dyes, stains, and pigments. Preferred colorants are pigments which may be combined with ingredients comprising the copolymer to interact with the D portion of the copolymer to form liquid toner compositions with structure as described herein, are at least nominally insoluble in and nonreactive with the carrier liquid, and are useful and effective in making visible the latent electrostatic image. It is understood that the visual enhancement additive(s) may also interact with each other physically and/or chemically, forming aggregations and/or agglomerates of visual enhancement additives that also interact with the D portion of the copolymer. Examples of suitable colorants include: phthalocyanine blue (C.I. Pigment Blue 15:1, 15:2, 15:3 and 15:4), monoarylide yellow (C.I. Pigment Yellow 1, 3, 65, 73 and 74), diarylide yellow (C.I. Pigment Yellow 12, 13, 14, 17 and 83), arylamide (Hansa) yellow (C.I. Pigment Yellow

23

10, 97, 105 and 111), isoindoline yellow (C.I. Pigment Yellow 138), azo red (C.I. Pigment Red 3, 17, 22, 23, 38, 48:1, 48:2, 52:1, and 52:179), quinacridone magenta (C.I. Pigment Red 122, 202 and 209), laked rhodamine magenta (C.I. Pigment Red 81:1, 81:2, 81:3, and 81:4), and black pigments such as finely divided carbon (Cabot Monarch 120, Cabot Regal 300R, Cabot Regal 350R, Vulcan X72, and Aztech ED 8200), and the like.

In addition to the visual enhancement additive, other additives optionally can be formulated into the liquid toner composition. A particularly preferred additive comprises at least one charge control agent (CCA, charge control additive or charge director). The charge control agent, also known as a charge director, can be included as a separate ingredient and/or included as one or more functional moiety(ies) of the S and/or D material incorporated into the amphipathic copolymer. The charge control agent acts to enhance the chargeability and/or impart a charge to the toner particles. Toner particles can obtain either positive or negative charge depending upon the combination of particle material and charge control agent.

The charge control agent can be incorporated into the toner particles using a variety of methods, such as copolymerizing a suitable monomer with the other monomers used to form the copolymer, chemically reacting the charge control agent with the toner particle, chemically or physically adsorbing the charge control agent onto the toner particle (resin or pigment), or chelating the charge control agent to a functional group incorporated into the toner particle. One preferred method is via a functional group built into the S material of the copolymer.

The charge control agent acts to impart an electrical charge of selected polarity onto the toner particles. Any number of charge control agents described in the art can be used. For example, the charge control agent can be provided in the form of metal salts consisting of polyvalent metal ions and organic anions as the counterion. Suitable metal ions include, but are not limited to, Ba(II), Ca(II), Mn(II), Zn(II), Zr(IV), Cu(II), Al(III), Cr(III), Fe(II), Fe(III), Sb(III), Bi(III), Co(II), La(III), Pb(II), Mg(II), Mo(III), Ni(II), Ag(I), Sr(II), Sn(IV), V(V), Y(III), and Ti(IV). Suitable organic anions include carboxylates or sulfonates derived from aliphatic or aromatic carboxylic or sulfonic acids, preferably aliphatic fatty acids such as stearic acid, behenic acid, neodecanoic acid, diisopropylsalicylic acid, octanoic acid, abietic acid, naphthenic acid, lauric acid, tallic acid, and the like.

Preferred negative charge control agents are lecithin and basic barium petronate. Preferred positive charge control agents include metallic carboxylates (soaps), for example, as described in U.S. Pat. No. 3,411,936 (incorporated herein by reference). A particularly preferred positive charge control agent is zirconium tetraoctoate (available as Zirconium HEX-CEM from OMG Chemical Company, Cleveland, Ohio).

The preferred charge control agent levels for a given toner formulation will depend upon a number of factors, including the composition of the S portion and the organosol, the molecular weight of the organosol, the particle size of the organosol, the D:S ratio of the polymeric binder, the pigment used in making the toner composition, and the ratio of organosol to pigment. In addition, preferred charge control agent levels will depend upon the nature of the electrophotographic imaging process. The level of charge control agent can be adjusted based upon the parameters listed herein, as known in the art. The amount of the charge control agent,

24

based on 100 parts by weight of the toner solids, is generally in the range of 0.01 to 10 parts by weight, preferably 0.1 to 5 parts by weight.

The conductivity of a liquid toner composition can be used to describe the effectiveness of the toner in developing electrophotographic images. A range of values from  $1 \times 10^{-11}$  mho/cm to  $3 \times 10^{-10}$  mho/cm is considered advantageous to those of skill in the art. High conductivities generally indicate inefficient association of the charges on the toner particles and is seen in the low relationship between current density and toner deposited during development. Low conductivities indicate little or no charging of the toner particles and lead to very low development rates. The use of charge control agents matched to adsorption sites on the toner particles is a common practice to ensure sufficient charge associates with each toner particle.

Other additives may also be added to the formulation in accordance with conventional practices. These include one or more of UV stabilizers, mold inhibitors, bactericides, fungicides, antistatic agents, gloss modifying agents, other polymer or oligomer material, antioxidants, and the like.

The particle size of the resultant charged toner particles can impact the imaging, fusing, resolution, and transfer characteristics of the toner composition incorporating such particles. Preferably, the volume mean particle diameter (determined with laser diffraction) of the particles is in the range of about 0.05 to about 50.0 microns, more preferably in the range of about 3 to about 10 microns, most preferably in the range of about 1.5 to about 5 microns.

In electrophotographic and electrographic processes, an electrostatic image is formed on the surface of a photoreceptive element or dielectric element, respectively. The photoreceptive element or dielectric element may be an intermediate transfer drum or belt or the substrate for the final toned image itself, as described by Schmidt, S. P. and Larson, J. R. in *Handbook of Imaging Materials* Diamond, A. S., Ed: Marcel Dekker: New York; Chapter 6, pp 227-252, and U.S. Pat. Nos. 4,728,983, 4,321,404, and 4,268,598.

In electrography, a latent image is typically formed by (1) placing a charge image onto the dielectric element (typically the receiving substrate) in selected areas of the element with an electrostatic writing stylus or its equivalent to form a charge image, (2) applying toner to the charge image, and (3) fixing the toned image. An example of this type of process is described in U.S. Pat. No. 5,262,259. Images formed by the present invention may be of a single color or a plurality of colors. Multicolor images can be prepared by repetition of the charging and toner application steps.

In electrophotography, the electrostatic image is typically formed on a drum or belt coated with a photoreceptive element by (1) uniformly charging the photoreceptive element with an applied voltage, (2) exposing and discharging portions of the photoreceptive element with a radiation source to form a latent image, (3) applying a toner to the latent image to form a toned image, and (4) transferring the toned image through one or more steps to a final receptor sheet. In some applications, it is sometimes desirable to fix the toned image using a heated pressure roller or other fixing methods known in the art.

While the electrostatic charge of either the toner particles or photoreceptive element may be either positive or negative, electrophotography as employed in the present invention is preferably carried out by dissipating charge on a positively charged photoreceptive element. A positively-

charged toner is then applied to the regions in which the positive charge was dissipated using a dry toner development technique.

The substrate for receiving the image from the photoreceptive element can be any commonly used receptor material, such as paper, coated paper, polymeric films and primed or coated polymeric films. Polymeric films include polyesters and coated polyesters, polyolefins such as polyethylene or polypropylene, plasticized and compounded polyvinyl chloride (PVC), acrylics, polyurethanes, polyethylene/acrylic acid copolymer, and polyvinyl butyral. The polymer film may be coated or primed, e.g. to promote toner adhesion.

These and other aspects of the present invention are demonstrated in the illustrative examples that follow.

### EXAMPLES

#### Test Methods and Apparatus

In the following examples, percent solids of the copolymer solutions and the organosol and ink dispersions were determined gravimetrically using the Halogen Lamp Drying Method using a halogen lamp drying oven attachment to a precision analytical balance (Mettler Instruments, Inc., Highstown, N.J.). Approximately two grams of sample were used in each determination of percent solids using this sample dry down method.

In the practice of the invention, molecular weight is normally expressed in terms of the weight average molecular weight, while molecular weight polydispersity is given by the ratio of the weight average molecular weight to the number average molecular weight. Molecular weight parameters were determined with gel permeation chromatography (GPC) using tetrahydrofuran as the carrier solvent. Absolute weight average molecular weight were determined using a Dawn DSP-F light scattering detector (Wyatt Technology Corp., Santa Barbara, Calif.), while polydispersity was evaluated by ratioing the measured weight average molecular weight to a value of number average molecular weight determined with an Optilab 903 differential refractometer detector (Wyatt Technology Corp., Santa Barbara, Calif.).

Organosol and toner particle size distributions were determined by the Laser Diffraction Light Scattering Method using a Horiba LA-900 laser diffraction particle size analyzer (Horiba Instruments, Inc., Irvine, Calif.). Samples are diluted approximately 1/500 by volume and sonicated for one minute at 150 watts and 20 kHz prior to measurement. Particle size was expressed as both a number mean diameter ( $D_n$ ) and a volume mean diameter ( $D_v$ ) and in order to provide an indication of both the fundamental (primary) particle size and the presence of aggregates or agglomerates.

The liquid toner conductivity (bulk conductivity,  $k_b$ ) was determined at approximately 18 Hz using a Scientifica Model 627 conductivity meter (Scientifica Instruments, Inc., Princeton, N.J.). In addition, the free (liquid dispersant) phase conductivity ( $k_f$ ) in the absence of toner particles was also determined. Toner particles were removed from the liquid medium by centrifugation at 5° C. for 1-2 hours at 6,000 rpm (6,110 relative centrifugal force) in a Jouan MR1822 centrifuge (Winchester, Va.). The supernatant liquid was then carefully decanted, and the conductivity of this liquid was measured using a Scientifica Model 627 conductance meter. The percentage of free phase conductivity relative to the bulk toner conductivity was then determined as 100% ( $k_f/k_b$ ).

Toner particle electrophoretic mobility (dynamic mobility) was measured using a Matec MBS-8000 Electrokinetic

Sonic Amplitude Analyzer (Matec Applied Sciences, Inc., Hopkinton, Mass.). Unlike electrokinetic measurements based upon microelectro-phoresis, the MBS-8000 instrument has the advantage of requiring no dilution of the toner sample in order to obtain the mobility value. Thus, it was possible to measure toner particle dynamic mobility at solids concentrations actually preferred in printing. The MBS-8000 measures the response of charged particles to high frequency (1.2 MHz) alternating (AC) electric fields. In a high frequency AC electric field, the relative motion between charged toner particles and the surrounding dispersion medium (including counter-ions) generates an ultrasonic wave at the same frequency of the applied electric field. The amplitude of this ultrasonic wave at 1.2 MHz can be measured using a piezoelectric quartz transducer; this electrokinetic sonic amplitude (ESA) is directly proportional to the low field AC electrophoretic mobility of the particles. The particle zeta potential can then be computed by the instrument from the measured dynamic mobility and the known toner particle size, liquid dispersant viscosity, and liquid dielectric constant.

The charge per mass measurement (Q/M) was measured using an apparatus that consists of a conductive metal plate, a glass plate coated with Indium Tin Oxide (ITO), a high voltage power supply, an electrometer, and a personal computer (PC) for data acquisition. A 1% solution of ink was placed between the conductive plate and the ITO coated glass plate. An electrical potential of known polarity and magnitude was applied between the ITO coated glass plate and the metal plate, generating a current flow between the plates and through wires connected to the high voltage power supply. The electrical current was measured 100 times a second for 20 seconds and recorded using the PC. The applied potential causes the charged toner particles to migrate towards the plate (electrode) having opposite polarity to that of the charged toner particles. By controlling the polarity of the voltage applied to the ITO coated glass plate, the toner particles may be made to migrate to that plate.

The ITO coated glass plate was removed from the apparatus and placed in an oven for approximately 30 minutes at 50° C. to dry the plated ink completely. After drying, the ITO coated glass plate containing the dried ink film was weighed. The ink was then removed from the ITO coated glass plate using a cloth wipe impregnated with Norpar™ 12, and the clean ITO glass plate was weighed again. The difference in mass between the dry ink coated glass plate and the clean glass plate is taken as the mass of ink particles (m) deposited during the 20 second plating time. The electrical current values were used to obtain the total charge carried by the toner particles (Q) over the 20 seconds of plating time by integrating the area under a plot of current vs. time using a curve-fitting program (e.g. TableCurve 2D from Systat Software Inc.). The charge per mass (Q/M) was then determined by dividing the total charge carried by the toner particles by the dry plated ink mass.

In the following examples, toner was printed onto final image receptors using the following methodology (referred to in the Examples as the Liquid Electrophotographic Printing Method):

A light sensitive temporary image receptor (organic photoreceptor or "OPC") was charged with a uniform positive charge of approximately 850 volts. The positively charged surface of the OPC was image-wise irradiated with a scanning infrared laser module in order to reduce the charge wherever the laser struck the surface. Typical charge-reduced values were between 50 volts and 100 volts.

A developer apparatus was then utilized to apply the toner particles to the OPC surface. The developer apparatus included the following elements: a conductive rubber developer roll in contact with the OPC, liquid toner, a conductive deposition roll, an insulative foam cleaning roll in contact with developer roll surface, and a conductive skiving blade (skive) in contact with the developer roll. The contact area between the developer roll and the OPC is referred to as the "developing nip." The developer roll and conductive deposition roll were both partially suspended in the liquid toner. The developer roll delivered liquid toner to the OPC surface, while the conductive deposition roll was positioned with its roll axis parallel to the developer roll axis and its surface arranged to be approximately 150 microns from the surface of the developer roll, thereby forming a deposition gap.

During development, toner was initially transferred to the developer roll surface by applying a voltage of approximately 500 volts to the conductive developer roll and applying a voltage of 600 volts to the deposition roll. This created a 100-volt potential between the developer roll and the deposition roll so that in the deposition gap, toner particles (which were positively charged) migrated to the surface of the developer roll and remained there as the developer roll surface exited from the liquid toner into the air.

The conductive metal skive was biased to at least 600 volts (or more) and skived liquid toner from the surface of the developer roll without scraping off the toner layer that was deposited in the deposition gap. The developer roll surface at this stage contained a uniformly thick layer of toner at approximately 25% solids. As this toner layer passed through the developing nip, toner was transferred from the developer roll surface to the OPC surface in all the discharged areas of the OPC (the charge image), since the toner particles were positively charged. At the exit of the developing nip, the OPC contained a toner image and the developer roll contained a negative of that toner image which was subsequently cleaned from the developer roll surface by encountering the rotating foam cleaning roll.

The developed latent image (toned image) on the photoreceptor was subsequently transferred to the final image receptor without film formation of the toner on the OPC. Transfer was effected either directly to the final image receptor, or indirectly using an electrostatically-assisted offset transfer to an Intermediate Transfer Belt (ITB), with subsequent electrostatically-assisted offset transfer to the final image receptor. Smooth, clay coated papers were preferred final image receptors for direct transfer of a non-film formed toner from the photoreceptor, while plain, uncoated 20 pound bond paper was a preferred final image receptor for offset transfer using an electrostatic assist. Electrostatically-assisted transfer of non film-formed toner was most effective when the transfer potential (potential difference between the toner on the OPC and the paper back-up roller for direct transfer; or potential difference between the toner on the OPC and the ITB for offset transfer) was maintained in the range of 200–1000 V or 800–2000 V, respectively.

#### Materials

The following abbreviations are used in the examples:

BHA: Behenyl acrylate (a PCC available from Ciba Specialty Chemical Co., Suffolk, Va.)

BMA: Butyl methacrylate (available from Aldrich Chemical Co., Milwaukee, Wis.)

EMA: Ethyl methacrylate (available from Aldrich Chemical Co., Milwaukee, Wis.)

- Exp 61: Amine-functional silicone wax (a PCC available from Genesee Polymer Corporation, Flint, Mich.)
- HEMA: 2-Hydroxyethyl methacrylate (available from Aldrich Chemical Co., Milwaukee, Wis.)
- 5 LMA: Lauryl methacrylate (available from Aldrich Chemical Co., Milwaukee, Wis.)
- ODA: Octadecyl acrylate (a PCC available Aldrich Chemical Co., Milwaukee, Wis.)
- TCHMA: Trimethyl cyclohexyl methacrylate (available from Ciba Specialty Chemical Co., Suffolk, Va.)
- 10 St: Styrene (available from Aldrich Chemical Co., Milwaukee, Wis.)
- TMI: Dimethyl-m-isopropenyl benzyl isocyanate (available from CYTEC Industries, West Paterson, N.J.)
- 15 AIBN: Azobisisobutyronitrile (an initiator available as VAZO-64 from DuPont Chemical Co., Wilmington, Del.)
- V-601: Dimethyl 2,2'-azobisisobutyrate (an initiator available as V-601 from WAKO Chemicals U.S.A., Richmond, Va.)
- 20 DBTDL: Dibutyl tin dilaurate (a catalyst available from Aldrich Chemical Co., Milwaukee, Wis.)
- Zirconium HEX-CEM: (metal soap, zirconium tetraoctoate, available from OMG Chemical Company, Cleveland, Ohio)

#### 25 Nomenclature

In the following examples, the compositional details of each copolymer will be summarized by ratioing the weight percentages of monomers used to create the copolymer. The 30 grafting site composition is expressed as a weight percentage of the monomers comprising the copolymer or copolymer precursor, as the case may be. For example, a graft stabilizer (precursor to the S portion of the copolymer) is designated TCHMA/HEMA-TMI (97/3–4.7) is made by copolymerizing, on a relative basis, 97 parts by weight TCHMA and 3 parts by weight HEMA, and this hydroxy functional polymer was reacted with 4.7 parts by weight of TMI.

Similarly, a graft copolymer organosol designated 40 TCHMA/HEMA-TMI//EMA (97–3–4.7//100) is made by copolymerizing the designated graft stabilizer (TCHMA/HEMA-TMI (97/3–4.7)) (S portion or shell) with the designated core monomer EMA (D portion or core) at a specified ratio of D/S (core/shell) determined by the relative 45 weights reported in the examples.

#### Examples 1–5

##### Preparation of Copolymer S Materials, also Referred to Herein as "Graft Stabilizers"

###### Example 1 (Comparative)

A 5000 ml 3-neck round flask equipped with a condenser, 55 a thermocouple connected to a digital temperature controller, a nitrogen inlet tube connected to a source of dry nitrogen and a magnetic stirrer, was charged with a mixture of 2561 g of Norpar<sup>TM</sup> 15, 849 g of LMA, 26.7 g of 98% HEMA, and 8.31 g of AIBN. While stirring the mixture, the 60 reaction flask was purged with dry nitrogen for 30 minutes at flow rate of approximately 2 liters/minute. A hollow glass stopper was then inserted into the open end of the condenser and the nitrogen flow rate was reduced to approximately 0.5 liters/minute. The mixture was heated to 70° C. for 16 hours. 65 The conversion was quantitative.

The mixture was then heated to 90° C. and held at that temperature for 1 hour to destroy residual AIBN, then was

29

cooled back to 70° C. The nitrogen inlet tube was then removed, and 13.6 g of 95% DBTDL were added to the mixture, followed by 41.1 g of TMI. The TMI was added drop wise over the course of approximately 5 minutes while stirring the reaction mixture. The nitrogen inlet tube was replaced, the hollow glass stopper in the condenser was removed, and the reaction flask was purged with dry nitrogen for 30 minutes at a flow rate of approximately 2 liters/minute. The hollow glass stopper was reinserted into the open end of the condenser and the nitrogen flow rate was reduced to approximately 0.5 liters/minute. The mixture was allowed to react at 70° C. for 6 hours, at which time the conversion was quantitative.

The mixture was then cooled to room temperature. The cooled mixture was a viscous, transparent liquid containing no visible insoluble matter. The percent solids of the liquid mixture was determined to be 25.64% using the Halogen Lamp Drying Method described above. Subsequent determination of molecular weight was made using the GPC method described above; the copolymer had  $M_w$  of 231,350 Da and  $M_w/M_n$  of 3.2 based upon two independent measurements. The product is a copolymer of LMA and HEMA containing random side chains of TMI and is designated herein as LMA/HEMA-TMI (97/3-4.7% w/w), does not contain a PCC, and is suitable for making an organosol.

#### Example 2 (Comparative)

Using the method and apparatus of Example 1, 2561 g of Heptane, 849 g of TCHMA, 26.8 g of 98% HEMA and 8.31 g of V-601 were combined and resulting mixture reacted at 70° C. for 16 hours. The mixture was then heated to 90° C. for 1 hour to destroy any residual V-601, then was cooled back to 70° C. To the cooled mixture was then added 13.6 g of 95% DBTDL and 41.1 g of TMI. The TMI was added drop wise over the course of approximately 5 minutes while stirring the reaction mixture. Following the procedure of Example 1, the mixture was reacted at 70° C. for approximately 6 hours at which time the reaction was quantitative. The mixture was then cooled to room temperature. The cooled mixture was a viscous, transparent solution, containing no visible insoluble matter.

The percent solids of the liquid mixture was determined to be 28.86% using the Halogen Lamp Drying Method described above. Subsequent determination of molecular weight was made using the GPC method described above; the copolymer had a  $M_w$  of 301,000 Da and  $M_w/M_n$  of 3.3 based upon two independent measurements. The product was a copolymer of TCHMA and HEMA containing random side chains of TMI and was designated herein as TCHMA/HEMA-TMI (97/3-4.7% w/w), does not contain a PCC, and is suitable for making an organosol.

#### Example 3

Using the method and apparatus of Example 1, 2561 g of Norpar<sup>TM</sup> 12, 849 g of BHA, 26.8 g of 98% HEMA and 8.31 g of V-601 were combined and resulting mixture reacted at 70° C. for 16 hours. The mixture was then heated to 90° C. for 1 hour to destroy any residual V-601, then was cooled back to 70° C. To the cooled mixture was then added 13.6 g of 95% DBTDL and 41.1 g of TMI. The TMI was added drop wise over the course of approximately 5 minutes while stirring the reaction mixture. Following the procedure of Example 1, the mixture was reacted at 70° C. for approximately 6 hours at which time the reaction was quantitative. The mixture was then cooled to room temperature. The

30

cooled mixture was a viscous, transparent solution, containing no visible insoluble matter.

The percent solids of the liquid mixture was determined to be 26.25% using the Halogen Lamp Drying Method described above. Subsequent determination of molecular weight was made using the GPC method described above; the copolymer had a  $M_w$  of 248,650 Da and  $M_w/M_n$  of 2.9 based upon two independent measurements. The product was a copolymer of BHA and HEMA containing random side chains of TMI and was designated herein as BHA/HEMA-TMI (97/3-4.7% w/w), contains a PCC, and is suitable for making an organosol.

#### Example 4

Using the method and apparatus of Example 1, 2561 g of Norpar<sup>TM</sup> 12, 849 g of ODA, 26.8 g of 98% HEMA and 8.31 g of V-601 were combined and resulting mixture reacted at 70° C. for 16 hours. The mixture was then heated to 90° C. for 1 hour to destroy any residual V-601, then was cooled back to 70° C. To the cooled mixture was then added 13.6 g of 95% DBTDL and 41.1 g of TMI. The TMI was added drop wise over the course of approximately 5 minutes while stirring the reaction mixture. Following the procedure of Example 1, the mixture was reacted at 70° C. for approximately 6 hours at which time the reaction was quantitative. The mixture was then cooled to room temperature. The cooled mixture was a viscous, transparent solution, containing no visible insoluble matter.

The percent solids of the liquid mixture was determined to be 26.21% using the Halogen Lamp Drying Method described above. Subsequent determination of molecular weight was made using the GPC method described above; the copolymer had a  $M_w$  of 213,600 Da and  $M_w/M_n$  of 1.5 based upon two independent measurements. The product was a copolymer of ODA and HEMA containing random side chains of TMI and was designated herein as ODA/HEMA-TMI (97/3-4.7% w/w), contains a PCC, and is suitable for making an organosol.

#### Example 5 (Comparative)

Using the method and apparatus of Example 1, 2561 g of Norpar<sup>TM</sup> 15, 424 g of LMA, 414 g of TCHMA, 26.8 g of 98% HEMA, and 8.31 g of AIBN were combined and resulting mixture reacted at 70° C. for 16 hours. The mixture was then heated to 90° C. for 1 hour to destroy any residual AIBN, then was cooled back to 70° C. To the cooled mixture was then added 13.6 g of 95% DBTDL and 41.1 g of TMI. The TMI was added drop wise over the course of approximately 5 minutes while stirring the reaction mixture. Following the procedure of Example 1, the mixture was reacted at 70° C. for approximately 6 hours at which time the reaction was quantitative. The mixture was then cooled to room temperature. The cooled mixture was a viscous, transparent solution, containing no visible insoluble matter.

The percent solids of the liquid mixture was determined to be 25.76% using the Halogen Lamp Drying Method described above. Subsequent determination of molecular weight was made using the GPC method described above; the copolymer had a  $M_w$  of 181,110 Da and  $M_w/M_n$  of 1.9 based upon two independent measurements. The product was a copolymer of LMA, TCHMA and HEMA containing random side chains of TMI and was designated herein as LMA/TCHMA/HEMA-TMI (48.5/48.5/3-4.7% w/w), does not contain a PCC, and is suitable for making an organosol.

The compositions of the graft stabilizers of Examples 1–5 are summarized in the following table:

TABLE 2

| Graft Stabilizers (S portion)        |                        | Calculated Stabilizer<br>$T_g$<br>(° C.) | Solids<br>(%) | Molecular Weight |           |
|--------------------------------------|------------------------|------------------------------------------|---------------|------------------|-----------|
| Graft Stabilizer Composition         | Example Number (% w/w) |                                          |               | $M_w$ (Da)       | $M_w/M_n$ |
| LMA/HEMA-TMI (97/3-4.7)              | 1                      | -65                                      | 25.64         | 231,350          | 3.2       |
| TCHMA/HEMA-TMI (97/3-4.7)            | 2                      | 125                                      | 28.86         | 301,000          | 3.3       |
| BHA/HEMA-TMI (97/3-4.7)              | 3                      | <-55                                     | 26.25         | 248,650          | 2.9       |
| ODA/HEMA-TMI (97/3-4.7)              | 4                      | -55                                      | 26.21         | 213,600          | 1.5       |
| LMA/TCHMA/HEMA-TMI (48.5/48.5/3-4.7) | 5                      | 0                                        | 25.76         | 181,110          | 1.9       |

$T_g$  calculations exclude the HEMA-TMI grafting site

### Examples 6–15

#### Addition of D Material to Form Organosols

##### Example 6 (Comparative)

This is a comparative example using the graft stabilizer in Example 1 to prepare an organosol that does not incorporate a PCC. A 5000 ml 3-neck round flask equipped with a condenser, a thermocouple connected to a digital temperature controller, a nitrogen inlet tube connected to a source of dry nitrogen and a magnetic stirrer, was charged with a mixture of 2943 g of Norpar<sup>TM</sup> 12, 373 g of EMA, 180 g of the graft stabilizer mixture from Example 1 at 25.64% polymer solids, and 6.3 g of AIBN. While stirring the mixture, the reaction flask was purged with dry nitrogen for 30 minutes at flow rate of approximately 2 liters/minute. A hollow glass stopper was then inserted into the open end of the condenser and the nitrogen flow rate was reduced to approximately 0.5 liters/minute. The mixture was heated to 70° C. for 16 hours. The conversion was quantitative.

The resulting mixture was stripped of residual monomer using a rotary evaporator equipped with a dry ice/acetone condenser and operating at a temperature of 90° C. and a vacuum of approximately 15 mm Hg. The stripped organosol was cooled to room temperature, yielding an opaque white dispersion.

This organosol was designated LMA/HEMA-TMI//EMA (97/3–4.7//100% w/w), and can be used to prepare a liquid toner that does not contain a PCC in the binder. The percent solids of the organosol dispersion after stripping was determined as 14.83% using the Halogen Lamp Drying Method described above. Subsequent determination of average particle size was made using the Laser Diffraction Light Scattering Method described above; the organosol had a volume average diameter of 23.4  $\mu$ m.

##### Example 7 (Comparative)

This is an example using the graft stabilizer in Example 2 to prepare an organosol that does not incorporate a PCC. Using the method and apparatus of Example 6, 2534 g of Heptane, 528 g of EMA, 229 g of the graft stabilizer mixture from Example 2 at 28.86% polymer solids, and 8.9 g of V-601 were combined. The mixture was heated to 70° C. for

16 hours. The conversion was quantitative. The mixture then was cooled to room temperature. After stripping the orga-

nosol using the method of Example 6 to remove residual monomer, the stripped organosol was cooled to room temperature, yielding an opaque white dispersion.

This organosol was designated TCHMA/HEMA-TMI//EMA (97/3–4.7//100% w/w), and can be used to prepare a liquid toner that does not contain a PCC in the binder. The percent solids of the organosol dispersion after stripping was determined as 22.49% using the Halogen Lamp Drying Method described above. Subsequent determination of average particle size was made using the Laser Diffraction Light Scattering Method described above; the organosol had a volume average diameter of 0.47  $\mu$ m.

##### Example 8

This is an example using the graft stabilizer in Example 3 to prepare an organosol that contains a PCC in the S portion of the organosol. Using the method and apparatus of Example 6, 2838 g of Norpar<sup>TM</sup> 12,336 g of EMA, 320 g of the graft stabilizer mixture from Example 3 at 26.25% polymer solids, and 6.30 g of V-601 were combined. The mixture was heated to 70° C. for 16 hours. The conversion was quantitative. The mixture then was cooled to room temperature. After stripping the organosol using the method of Example 6 to remove residual monomer, the stripped organosol was cooled to room temperature, yielding an opaque white dispersion.

This organosol was designated BHA/HEMA-TMI//EMA (97/3–4.7//100% w/w), and can be used to prepare a liquid toner that contains a PCC in the binder. The percent solids of the organosol dispersion after stripping was determined as 11.79% using the Halogen Lamp Drying Method described above. Subsequent determination of average particle size was made using the Laser Diffraction Light Scattering Method described above; the organosol had a volume average diameter of 41.4  $\mu$ m.

##### Example 9

This is an example using the graft stabilizer in Example 3 to prepare an organosol that contains a PCC in the S portion of the organosol. Using the method and apparatus of Example 6, 2838 g of Norpar<sup>TM</sup> 12,336 g of Styrene, 320 g of the graft stabilizer mixture from Example 3 at 26.25% polymer solids, and 6.30 g of V-601 were combined. The mixture was heated to 70° C. for 16 hours. The conversion

was quantitative. The mixture then was cooled to room temperature. After stripping the organosol using the method of Example 6 to remove residual monomer, the stripped organosol was cooled to room temperature, yielding an opaque white dispersion.

This organosol was designated BHA/HEMA-TMI//St (97/3-4.7//100% w/w), and can be used to prepare a liquid toner that contains a PCC in the binder. The percent solids of the organosol dispersion after stripping was determined as 12.00% using the Halogen Lamp Drying Method described above. Subsequent determination of average particle size was made using the Laser Diffraction Light Scattering Method described above; the organosol had a volume average diameter of 1.2  $\mu\text{m}$ .

#### Example 10

This is an example using the graft stabilizer in Example 4 to prepare an organosol that contains a PCC in the S portion of the organosol. Using the method and apparatus of Example 6, 2837 g of Norpar<sup>TM</sup> 12, 336 g of BMA, 320 g of the graft stabilizer mixture from Example 4 at 26.21% polymer solids, and 6.30 g of V-601 were combined. The mixture was heated to 70° C. for 1.6 hours. The conversion was quantitative. The mixture then was cooled to room temperature. After stripping the organosol using the method of Example 6 to remove residual monomer, the stripped organosol was cooled to room temperature, yielding an opaque white dispersion.

This organosol was designated ODA/HEMA-TMI//BMA (97/3-4.7//100% w/w), and can be used to prepare a liquid toner that contains a PCC in the binder. The percent solids of the organosol dispersion after stripping was determined as 11.69% using the Halogen Lamp Drying Method described above. Subsequent determination of average particle size was made using the Laser Diffraction Light Scattering Method described above; the organosol had a volume average diameter of 1.1  $\mu\text{m}$ .

#### Example 11

This is an example using the graft stabilizer in Example 4 to prepare an organosol that contains a PCC in the S portion of the organosol. Using the method and apparatus of Example 6, 2837 g of Norpar<sup>TM</sup> 12, 336 g of EMA, 320 g of the graft stabilizer mixture from Example 4 at 26.21% polymer solids, and 6.30 g of V-601 were combined. The mixture was heated to 70° C. for 16 hours. The conversion was quantitative. The mixture then was cooled to room temperature. After stripping the organosol using the method of Example 6 to remove residual monomer, the stripped organosol was cooled to room temperature, yielding an opaque white dispersion.

This organosol was designated ODA/HEMA-TMI//EMA (97/3-4.7//100% w/w), and can be used to prepare a liquid toner that contains a PCC in the binder. The percent solids of the organosol dispersion after stripping was determined as 13.76% using the Halogen Lamp Drying Method described above. Subsequent determination of average particle size was made using the Laser Diffraction Light Scattering Method described above; the organosol had a volume average diameter of 45.6  $\mu\text{m}$ .

#### Example 12

This is an example using a silicone to prepare an organosol that contains a PCC in the S portion of the organosol.

Using the method and apparatus of Example 6, 3066 g of Norpar<sup>TM</sup> 12, 84 g of Exp61 (available from Genesee Polymers Corporation), and 8.4 g of TMI were mixed and heated to 45° C. for 6 hours. Then 336 g of EMA and 6.30 g of V-601 were added. The mixture was heated to 70° C. for 16 hours. The conversion was quantitative. The mixture then was cooled to room temperature. After stripping the organosol using the method of Example 6 to remove residual monomer, the stripped organosol was cooled to room temperature, yielding an opaque white dispersion.

This organosol was designated Exp61-TMI//EMA (91-9//100% w/w), and can be used to prepare a liquid toner that contains a PCC in the binder. The percent solids of the organosol dispersion after stripping was determined as 14.17% using the Halogen Lamp Drying Method described above. Subsequent determination of average particle size was made using the Laser Diffraction Light Scattering Method described above; the organosol had a volume average diameter of 1.8  $\mu\text{m}$ .

#### Example 13

This is an example using the graft stabilizer in Example 1 to prepare an organosol that contains a PCC in the D portion of the organosol. Using the method and apparatus of Example 6, 2941 g of Norpar<sup>TM</sup> 15, 298 g of EMA, 75 g of BHA, 180 g of the graft stabilizer mixture from Example 1 at 25.64% polymer solids, and 6.30 g AIBN were combined. The mixture was heated to 70° C. for 16 hours. The conversion was quantitative. The mixture then was cooled to room temperature. After stripping the organosol using the method of Example 6 to remove residual monomer, the stripped organosol was cooled to room temperature, yielding an opaque white dispersion.

This organosol was designated LMA/HEMA-TMI//EMA/BHA (97/3-4.7//80/20% w/w), and can be used to prepare a liquid toner that contains a PCC in the binder. The percent solids of the organosol dispersion after stripping was determined as 12.58% using the Halogen Lamp Drying Method described above. Subsequent determination of average particle size was made using the Laser Diffraction Light Scattering Method described above; the organosol had a volume average diameter of 159  $\mu\text{m}$ .

#### Example 14

This is an example using the graft stabilizer in Example 1 to prepare an organosol that contains a PCC in the D portion of the organosol. Using the method and apparatus of Example 6, 2941 g of Norpar<sup>TM</sup> 15, 298 g of EMA, 75 g of ODA, 180 g of the graft stabilizer mixture from Example 1 at 25.64% polymer solids, and 6.30 g AIBN were combined. The mixture was heated to 70° C. for 16 hours. The conversion was quantitative. The mixture then was cooled to room temperature. After stripping the organosol using the method of Example 6 to remove residual monomer, the stripped organosol was cooled to room temperature, yielding an opaque white dispersion.

This organosol was designated LMA/HEMA-TMI//EMA/ODA (97/3-4.7//80/20% w/w), and can be used to prepare a liquid toner that contains a PCC in the binder. The percent solids of the organosol dispersion after stripping was determined as 10.59% using the Halogen Lamp Drying Method described above. Subsequent determination of average particle size was made using the Laser Diffraction Light Scattering Method described above; the organosol had a volume average diameter of 39  $\mu\text{m}$ .

This is an example using the graft stabilizer in Example 5 to prepare an organosol that contains a PCC in the D portion of the organosol. Using the method and apparatus of Example 6, 2941 g of Norpar<sup>TM</sup> 12, 298 g of EMA, 74.6 g of BHA, 180 g of the graft stabilizer mixture from Example 5 at 25.76% polymer solids, and 6.30 g AIBN were combined. The mixture was heated to 70° C. for 16 hours. The conversion was quantitative. The mixture then was cooled to room temperature. After stripping the organosol using the method of Example 6 to remove residual monomer, the stripped organosol was cooled to room temperature, yielding an opaque white dispersion.

This organosol was designated LMA/TCHMA/HEMA-TMI//EMA/BHA (48.5/48.5/3-4.7//80/20% w/w), and can be used to prepare a liquid toner that contains a PCC in the binder. The percent solids of the organosol dispersion after stripping was determined as 15.99% using the Halogen Lamp Drying Method described above. Subsequent determination of average particle size was made using the Laser Diffraction Light Scattering Method described above; the organosol had a volume average diameter of 28.6  $\mu$ m.

The compositions of the organosol copolymers formed in Examples 6-15 are summarized in the following table:

TABLE 3

| Example Number  | Organosol Copolymer Composition (% w/w)              | Calculated                    |                         |
|-----------------|------------------------------------------------------|-------------------------------|-------------------------|
|                 |                                                      | Core (D Portion) $T_g$ (° C.) | Calculated $T_g$ (° C.) |
| (Comparative) 6 | LMA/HEMA-TMI//EMA (97/3-4.7//100)                    | 65                            | 41                      |
| (Comparative) 7 | TCHMA/HEMA-TMI//EMA (97/3-4.7//100)                  | 65                            | 71                      |
| 8               | BHA/HEMA-TMI//EMA (97/3-4.7//100)                    | 65                            | *                       |
| 9               | BHA/HEMA-TMI//St (97/3-4.7//100)                     | 100                           | *                       |
| 10              | ODA/HEMA-TMI//BMA (97/3-4.7//100)                    | 20                            | 8                       |
| 11              | ODA/HEMA-TMI//EMA (97/3-4.7//100)                    | 65                            | 43                      |
| 12              | Silicone Wax (Exp61)-TMI//EMA (91/9//100)            | 65                            | *                       |
| 13              | LMA/HEMA-TMI//EMA/BHA (97/3-4.7//80/20)              | <65                           | *                       |
| 14              | LMA/HEMA-TMI//EMA/ODA (97/3-4.7//80/20)              | 31                            | 15                      |
| 15              | LMA/TCHMA/HEMA-TMI//EMA/BHA (48.5/48.5/3-4.7//80/20) | <65                           | *                       |

\*Not calculated, contains BHA or Exp61 PCC

## Examples 16-19

## Preparation of Liquid Toners

For characterization of the prepared liquid toner compositions in these examples, the following were measured: size-related properties (particle size); charge-related properties (bulk and free phase conductivity, dynamic mobility and zeta potential); and charge/developed reflectance optical density (Z/ROD), a parameter that is directly proportional to the toner charge/mass (Q/M).

This is an example of preparing a magenta liquid toner at a weight ratio of organosol copolymer to pigment of 5 (O/P ratio) using the organosol prepared in Example 13, for which the weight ratio of D material to S material was 8. 238 g of the organosol at 12.58% (w/w) solids in Norpar<sup>TM</sup> 15 were combined with 55 g of Norpar<sup>TM</sup> 15, 6 g of Pigment Red 81:4 (1Y-0001-9951-A, Magruder Color Company, Tucson, Ariz.) and 1.02 g of 5.91% Zirconium HEX-CEM solution (OMG Chemical Company, Cleveland, Ohio) in an 8 ounce glass jar. This mixture was then milled in a 0.5 liter vertical bead mill (Model 6TSG-1/4, Amex Co., Led., Tokyo, Japan) and charged with 390 g of 1.3 mm diameter Potters glass beads (Potters Industries, Inc., Parsippany, N.J.). The mill was operated at 2,000 RPM for 1.5 hours without cooling water circulating through the cooling jacket of the milling chamber.

A 12% (w/w) solids toner concentrate exhibited the following properties as determined using the test methods described above:

Volume Mean Particle Size: 4.5 micron  
Q/M: 323  $\mu$ C/g  
Bulk Conductivity: 327 picoMhos/cm  
Percent Free Phase Conductivity: 31%  
Dynamic Mobility: 3.65E-11 (m<sup>2</sup>/Vsec).

This toner was tested using the Liquid Electrophotographic Printing Method described previously. The reflection optical density (ROD) was 1.3 at plating voltages greater than 450 volts.

## Example 17

This is an example of preparing a black liquid toner at a weight ratio of organosol copolymer to pigment of 6 (O/P ratio) using the organosol prepared in Example 13, for which the weight ratio of D material to S material was 8.245 g of the organosol at 12.58% (w/w) solids in Norpar<sup>TM</sup> 15 were combined with 49 g of Norpar<sup>TM</sup> 15, 65 g of Black pigment (Aztech EK8200, Magruder Color Company, Tucson, Ariz.) and 0.87 g of 5.91% Zirconium HEX-CEM solution (OMG Chemical Company, Cleveland, Ohio) in an 8 ounce glass jar. This mixture was then milled in a 0.5 liter vertical bead mill (Model 6TSG-1/4, Amex Co., Led., Tokyo, Japan) and charged with 390 g of 1.3 mm diameter Potters glass beads (Potters Industries, Inc., Parsippany, N.J.). The mill was operated at 2,000 RPM for 1.5 hours without cooling water circulating through the cooling jacket of the milling chamber.

A 12% (w/w) solids toner concentrate exhibited the following properties as determined using the test methods described above:

Volume Mean Particle Size: 3.1 micron  
Q/M: 646  $\mu$ C/g  
Bulk Conductivity: 574 picoMhos/cm  
Percent Free Phase Conductivity: 29.9%  
Dynamic Mobility: 5.49E-11 (m<sup>2</sup>/Vsec)

This toner was tested on using the Liquid Electrophotographic Printing Method described previously. The reflection optical density (ROD) was 1.0 at plating voltages greater than 450 volts.

## Example 18

This is an example of preparing a cyan liquid toner at a weight ratio of organosol copolymer to pigment of 8 (O/P

ratio) using the organosol prepared in Example 13, for which the weight ratio of D material to S material was 8. 254 g of the organosol at 12.58% (w/w) solids in Norpar<sup>TM</sup> 15 were combined with 41 g of Norpar<sup>TM</sup> 15, 4 g of Pigment Blue 15:4, 249-3450. Sun Chemical Company, Cincinnati, Ohio) and 0.68 of 5.91% Zirconium HEX-CEM solution (OMG Chemical Company, Cleveland, Ohio) in an 8 ounce glass jar. This mixture was then milled in a 0.5 liter vertical bead mill (Model 6TSG-1/4, Amex Co., Led., Tokyo, Japan) and charged with 390 g of 1.3 mm diameter Potters glass beads (Potters Industries, Inc., Parsippany, N.J.). The mill was operated at 2,000 RPM for 1.5 hours without cooling water circulating through the cooling jacket of the milling chamber.

A 12% (w/w) solids toner concentrate exhibited the following properties as determined using the test methods described above:

Volume Mean Particle Size: 3.7 micron

Q/M: 505  $\mu$ C/g

Bulk Conductivity: 100 picoMhos/cm

Percent Free Phase Conductivity: 3.4%

Dynamic Mobility: 1.81E-11 ( $m^2/Vsec$ )

This toner was tested on using the Liquid Electrophotographic Printing Method described previously. The reflection optical density (ROD) was 1.3 at plating voltages greater than 450 volts.

#### Example 19

This is an example of preparing a yellow liquid toner at a weight ratio of copolymer to pigment of 5 (O/P ratio) using the organosol prepared in Example 13, for which the weight ratio of D material to S material was 8. 238 g of the organosol at 12.58% (w/w) solids in Norpar<sup>TM</sup> 15 were combined with 53 g of Norpar<sup>TM</sup> 15, 4.8 g of Pigment Yellow 138, 1.2 g of Pigment Yellow 83 (Sun Chemical Company, Cincinnati, Ohio) and 2.54 g of 5.91% Zirconium HEX-GEM solution (OMG Chemical Company, Cleveland, Ohio) in an 8 ounce glass jar. This mixture was then milled in a 0.5 liter vertical bead mill (Model 6TSG-1/4, Amex Co., Led., Tokyo, Japan) and charged with 390 g of 1.3 mm diameter Potters glass beads (Potters Industries, Inc., Parsippany, N.J.). The mill was operated at 2,000 RPM for 1.5 hours without cooling water circulating through the cooling jacket of the milling chamber.

A 12% (w/w) solids toner concentrate exhibited the following properties as determined using the test methods described above:

Volume Mean Particle Size: 3.5 micron

Q/M: 347  $\mu$ C/g

Bulk Conductivity: 153 picoMhos/cm

Percent Free Phase Conductivity: 8.2%

Dynamic Mobility: 2.67E-11 ( $m^2/Vsec$ )

This toner was tested on using the Liquid Electrophotographic Printing Method described previously. The reflection optical density (ROD) was 0.8 at plating voltages greater than 450 volts.

The following table summarizes the liquid toner compositions prepared in Examples 16-19:

TABLE 4

| Liquid Electrographic Toners Incorporating Copolymers Derived from an Organosol Incorporating a PCC in the D Portion of the Copolymer (Using LMA/HEMA-TMI//EMA/BHA 97/3-4,7//80/20) |       |              |                       |                     |                              |                             |
|-------------------------------------------------------------------------------------------------------------------------------------------------------------------------------------|-------|--------------|-----------------------|---------------------|------------------------------|-----------------------------|
| Exam-<br>ple                                                                                                                                                                        | Color | O/P<br>Ratio | CCA<br>(mg/g pigment) | Q/M<br>( $\mu$ C/g) | D <sub>v</sub><br>( $\mu$ m) | ROD (at<br>$\geq 450$ devV) |
| 10                                                                                                                                                                                  | 16    | M            | 5                     | 10                  | 323                          | 4.5                         |
|                                                                                                                                                                                     | 17    | K            | 6                     | 10                  | 646                          | 3.1                         |
|                                                                                                                                                                                     | 18    | C            | 8                     | 10                  | 505                          | 3.7                         |
|                                                                                                                                                                                     | 19    | Y            | 5                     | 25                  | 347                          | 3.5                         |

#### Example 20 (Comparative)

#### Electrophotographic Printing, Fusing Properties and Image Durability for Cyan Organosol Toner without PCC in Copolymer

This is an example of preparing a pigmented Cyan toner from an organosol incorporating a copolymer that does not include a PCC. The organosol of Example 6, for which the ratio of D material to S material was 8, was used at a weight ratio of organosol copolymer to pigment of 5. 1.02 g of 5.91% Zirconium HEX-CEM solution (OMG Chemical Company, Cleveland, Ohio) was added to the organosol and pigment mixture in an 8 ounce glass jar. This mixture was then milled in a 0.5 liter vertical bead mill (Model 6TSG-1/4, Amex Co., Led., Tokyo, Japan) and charged with 390 g of 1.3 mm diameter Potters glass beads (Potter Industries, Inc., Parsippany, N.J.). The mill was operated at 2,000 RPM for 1.5 hours without cooling water circulating through the cooling jacket of the milling chamber.

The resultant toner was printed onto bond paper using the Liquid Electrophotographic Printing Method as previously described. The toned image was transferred to plain bond paper and dried for fifteen minutes at room temperature. The resulting toned images, comprising unfused toner particles on bond paper, were subsequently fused offline by passing the printed pages through the heated and pressurized nip of a two roller fuser assembly at 65 lb/in<sup>2</sup> and 14.5 inches/minute linear speed. Two different types of fuser rollers were used: a compliant Teflon<sup>®</sup> coated roller and a compliant silicone rubber coated roller. Fusing was carried out at temperatures of 150° C., 175° C., and 200° C.

The resulting fused images at each temperature, along with an unfused image, were subjected to the thermoplastic adhesive blocking test by storing images ink to paper (Adhesion test) or ink to ink (Cohesion test) for 24 hours at 58° C. and 75% relative humidity as described in ASTM Test Method D1146-88. Image Blocking Resistance is reported as "NO" if no image damage or image sticking was observed at the conclusion of the test, "VS" if very slight image damage or sticking was observed at the conclusion of the test, or "YES" if extensive image damage or sticking was observed at the conclusion of the test.

Image durability was also evaluated by measuring the reduction in the reflectance optical density for a solid developed image area on the final receptor after abrading for twenty passes in one direction using a standard white linen cloth fixed to the moving arm of a Crockmeter. The initial optical density (ROD) of the fused dry toner solid image on each page was first measured. After abrading for twenty passes in one direction using the white linen cloth, the increase in reflectance optical density on the cloth due to the

presence of abraded toner (CROD) was measured. The Erasure Resistance was then calculated according to the following formula:

$$\text{Erasure Resistance (\%)} = 100\% * \frac{[(\text{ROD} - \text{CROD})]}{\text{ROD}}$$

Erasure Resistance ranges between 0% (poor image durability) to 100% (excellent image durability; with higher Erasure Resistance percentages corresponding to better image durability after fusing at a given temperature.

The results of the Image Blocking tests, both Adhesion and Cohesion, as well as Erasure Resistance measurements, are summarized in Table 5 for the fused liquid toner images below.

#### Example 21

##### Electrophotographic Printing, Fusing Properties and Image Durability for Cyan Organosol Toner Incorporating PCC in the D Portion of the Copolymer

This is an example of preparing a pigmented Cyan toner from an organosol incorporating a copolymer that includes a PCC (ODA) in the D portion (core) of the copolymer.

Using the method and apparatus of Example 1, 2561 g of Norpar<sup>TM</sup> 12, 849 g of LMA, 26.8 g of 98% HEMA, and 8.75 g of V-601 were combined and resulting mixture reacted at 70° C. for 16 hours. The mixture was then heated to 90° C. for 1 hour to destroy residual V-601, then was cooled back to 70° C. To the cooled mixture was then added 13.6 g of 95% DBTDL and 41.1 g of TMI. The TMI was added drop wise over the course of approximately 5 minutes while stirring the reaction mixture. Following the procedure of Example 1, the mixture was reacted at 70° C. for approximately 6 hours at which time the reaction was quantitative. The mixture was then cooled to room temperature.

The cooled mixture was a viscous, transparent solution, containing no visible insoluble matter. The percent solids of the liquid mixture was determined to be 26.29% using the Halogen Drying Method described above. Subsequent determination of molecular weight was made using the GPC method described above; the copolymer had a  $M_w$  of 231, 850 Da and  $M_w/M_n$  of 2.72 based upon two independent measurements. The product was a copolymer of LMA, and HEMA containing random side chains of TMI and was designated herein as LMA/HEMA-TMI (97/3-4.7%) and was used to make an organosol which contains a PCC in the D portion of the organosol.

Using the method and apparatus of Example 6, 2943 g of Norpar<sup>TM</sup> 12, 298 g of EMA, 75 g of ODA, 178 g of the

above graft stabilizer copolymer at 26.29% polymer solids, and 6.3 g of V-601 were combined. The mixture was heated to 70° C. for 16 hours. The conversion was quantitative. The mixture then was cooled to room temperature. After stripping the organosol using the method of Example 6 to remove residual monomer, the stripped organosol was cooled to room temperature, yielding an opaque white dispersion. This organosol was designated LMA/HEMA-TMI//EMA/ODA (97/3-4.7//80/20%) and can be used to prepare liquid toner compositions. The percent solids of the gel organosol dispersion after stripping was determined as 13.75% using the Halogen Drying Method described above. Subsequent determination of average particle size was made using the Laser Diffraction Analysis described above; the organosol had a volume average diameter of 20.4  $\mu\text{m}$ .

The organosol, for which the ratio of D material to S material was 8, was combined with a pigment at a weight ratio of organosol copolymer to pigment of 8. 227 g of the organosol prepared above at 13.75% solids in Norpar<sup>TM</sup> 12, was combined with 69 g of Norpar<sup>TM</sup> 12, 4 g of Pigment Blue 15:4 (Sun Chemical Company, Cincinnati, Ohio) and 0.66 g of 5.91% Zirconium HEX-CEM solution (OMG Chemical Company, Cleveland, Ohio) in an 8 ounce glass jar. This mixture was then milled in a 0.5 liter vertical bead mill (Model 6TSG-1/4, Amex Co., Ltd., Tokyo, Japan) and charged with 390 g of 1.3 mm diameter Potters glass beads (Potters Industries, Inc., Parsippany, N.J.). The mill was operated at 2,000 RPM for 1.5 hours without cooling water circulating through the cooling jacket of the milling chamber.

The resultant toner was printed onto bond paper using the method described in Example 20. The toned image was transferred to plain hood paper and dried for fifteen minutes at room temperature. The resulting toned images, comprising unfused dried toner particles on bond paper, were subsequently fused offline by passing the printed pages through the heated and pressurized nip of a two roller fuser assembly at 65 lb./in<sup>2</sup> and 14.5 inches/minute linear speed. Two different types of fuser rollers were used: a compliant Teflon<sup>®</sup> coated roller and a compliant silicone rubber coated roller. Fusing was carried out at temperatures of 150° C., 175° C., and 200° C.

The resulting images fused at each temperature, along with an unfused image, were subjected to the Image Blocking Resistance and Erasure Resistance tests according to the methods of Example 20. The results of the Image Blocking tests, both Adhesion and Cohesion, as well as Erasure Resistance measurements, are summarized in Table 5 for these fused dry toner images:

TABLE 5

Comparative Fusing Properties, Erasure and Blocking Resistance of Printed Images for Cyan Organosol Toners With and Without PCC in D Portion (Core) of the Copolymer

| Organosol Copolymer Composition Used in Making             | Calculated Copolymer | Fuser Roller Temperature | Erasure Resistance (%) | Image Blocking Resistance |                |
|------------------------------------------------------------|----------------------|--------------------------|------------------------|---------------------------|----------------|
|                                                            |                      |                          |                        | 58° C. & 75% RH           | Adhesion       |
| Cyan Toner                                                 | $T_g$ (° C.)         | (° C.)                   | (%)                    | Image Blocking Resistance | Cohesion       |
| LMA/HEMA-TMI//EMA (no PCC in copolymer) (97/3-4.7//80/20%) | +41                  | UF<br>150<br>175         | 23.0<br>71.0<br>84.5   | NO<br>NO<br>NO            | NO<br>NO<br>NO |

TABLE 5-continued

Comparative Fusing Properties, Erasure and Blocking Resistance of Printed Images for Cyan Organosol Toners With and Without PCC in D Portion (Core) of the Copolymer

| Organosol Copolymer Composition Used in Making                          | Calculated Copolymer  | Fuser Roller Temperature | Erasure Resistance   | Image Blocking Resistance |                  |
|-------------------------------------------------------------------------|-----------------------|--------------------------|----------------------|---------------------------|------------------|
|                                                                         |                       |                          |                      | 58° C. & 75% RH           |                  |
| Cyan Toner                                                              | T <sub>g</sub> (° C.) | (° C.)                   | (%)                  | Adhesion                  | Cohesion         |
| Fused with Silicone Rolls                                               |                       | 200                      | 90.0                 | NO                        | NO               |
| LMA/HEMA-TMI//EMA (no PCC in copolymer) (97/3-4.7//100)                 | +41                   | UF 150                   | 23.0<br>fuser offset | NO<br>N/A                 | NO<br>N/A        |
| Fused with Teflon Rolls                                                 |                       | 175                      | fuser offset         | N/A                       | N/A              |
|                                                                         |                       | 200                      | fuser offset         | N/A                       | N/A              |
| LMA/HEMA-TMI//EMA/ODA (97/3-4.7//80/20) (PCC in D Portion of Copolymer) | +15                   | UF 150 175               | 75.0<br>83.2<br>86.0 | NO<br>NO<br>NO            | NO<br>NO<br>NO   |
| Fused w/-Silicone Rolls                                                 |                       | 200                      | 94.2                 | NO                        | NO               |
| LMA/HEMA-TMI//EMA/ODA (97/3-4.7//80/20) (PCC in D Portion of Copolymer) | +15                   | UF 150 175               | 75.0<br>91.3<br>86.0 | N/A<br>N/A<br>N/A         | N/A<br>NO<br>N/A |
| Fused with Teflon Roll                                                  |                       | 200                      | 86.8                 | N/A                       | N/A              |

\*UF = unfused

The data of Table 5 show the surprising effect that incorporation of a PCC into the copolymer has on the fusing performance of liquid toner particles derived from that copolymer. Toned images using toner incorporating the PCC exhibit higher Erasure Resistance in the unfused state and higher Erasure Resistance after fusing at any particular temperature in the range examined between 150–200° C. Liquid toner particles incorporating a PCC also exhibit acceptable erasure resistance values (Erasure Resistance greater than 80%) at fusing temperatures 25–50° C. lower than the comparable liquid toner not incorporating a PCC.

Other embodiments of this invention will be apparent to those skilled in the art upon consideration of this specification or from practice of the invention disclosed herein. Various omissions, modifications, and changes to the principles and embodiments described herein may be made by one skilled in the art without departing from the true scope and spirit of the invention which is indicated by the following claims. All patents, patent documents, and publications cited herein are hereby incorporated by reference as if individually incorporated.

What is claimed is:

1. A liquid electrophotographic toner composition comprising:
  - a liquid carrier having a Kauri-Butanol number less than 30 ml; and
  - a plurality of toner particles dispersed in the liquid carrier,

wherein the toner particles comprise at least one amphiphilic copolymer comprising one or more S material portions and one or more D material portions, wherein the S material portions and the D material portions have respective solubilities in the liquid carrier that are sufficiently different from each other such that the S material portions tend to be more solvated by the carrier while the D material portions tend to be more dispersed in the carrier, and wherein one or more of the D material portions comprises one or more polymerizable, crystallizable compounds.

2. The liquid electrophotographic toner composition according to claim 1, further comprising at least one visual enhancement additive.

3. The liquid electrophotographic toner composition according to claim 2, wherein the at least one visual enhancement additive comprises at least one pigment.

4. The liquid electrophotographic toner composition according to claim 2, wherein the one or more polymerizable, crystallizable compounds comprise a crystallizing polymeric moiety derived from a polymerizable monomer selected from the group consisting of alkylacrylates where the alkyl chain contains more than 13 carbon atoms and alkylmethacrylates where the alkyl chain contains more than 17 carbon atoms.

5. The liquid electrophotographic toner composition according to claim 4, wherein the polymerizable monomer is selected from the group consisting of hexacontanyl (meth) acrylate, pentacosanyl (meth)acrylate, behenyl (meth)acrylate, octadecyl (meth)acrylate, hexadecyl acrylate, and tetradecyl acrylate.

6. The liquid electrophotographic toner composition according to claim 2, wherein the one or more polymerizable, crystallizable compounds are present in an amount of up to 30% by weight of the D material.

7. The liquid electrophotographic toner composition according to claim 2, wherein the liquid carrier comprises a hydrocarbon.

8. The liquid electrophotographic toner composition according to claim 2, wherein the liquid carrier comprises an aliphatic hydrocarbon.

9. The liquid electrophotographic toner composition according to claim 2, further comprising one or more charge control agents.

10. The liquid electrophotographic toner composition according to claim 2, wherein the weight ratio of D material to S material is in the range of 2:1 to 10:1.

11. The liquid electrophotographic toner composition according to claim 2, wherein the amphiphilic copolymer has a graft structure comprising one or more D material portions grafted onto an S material portion.

12. A liquid electrophotographic toner composition comprising:

- a) a liquid carrier having a Kauri-Butanol number less than 30 ml; and
- b) a plurality of toner particles dispersed in the liquid carrier, wherein the toner particles comprise:
  - (i) one or more polymerizable, crystallizable compounds, and
  - (ii) at least one amphipathic copolymer comprising one or more S material portions and one or more D material portions, wherein the S material portions and the D material portions have respective solubilities in the liquid carrier that are sufficiently different from each other such that the S material portions tend to be more solvated by the carrier while the D material portions tend to be more dispersed in the carrier, wherein one or more of the D material portions comprises one or more polymerizable, crystallizable compounds, and wherein the D material portion has a glass transition temperature calculated according to the Fox equation of greater than 55° C.

13. The liquid electrophotographic toner composition according to claim 12 wherein one or more polymerizable, crystallizable compounds are located in the S portion of the copolymer.

14. A liquid electrophotographic toner composition comprising:

- a) a liquid carrier having a Kauri-Butanol number less than 30 ml; and
- b) a plurality of toner particles dispersed in the liquid carrier,

wherein the toner particles incorporate:

- (i) at least one amphipathic copolymer comprising one or more S material portions and one or more D material portions, wherein the S material portions and the D material portions have respective solubilities in the liquid carrier that are sufficiently different from each other such that the S material portions tend to be more solvated by the carrier while the D material portions tend to be more dispersed in the carrier, and
- (ii) one or more polymerizable, crystallizable compounds incorporated into the D material portion, or both the S material portion and the D material portion,

wherein the D material portion has a glass transition temperature calculated according to the Fox equation in the range of 30° C. to 50° C.

15. A method of making a liquid electrographic toner composition comprising steps of:

- a) providing an organosol comprising a plurality of toner particles dispersed in a liquid carrier, wherein the toner particles comprise at least one amphipathic copolymer, wherein the amphipathic copolymer comprises one or more S material portions and one or more D material portions, wherein the S material portions and the D material portions have respective solubilities in the liquid carrier that are sufficiently different from each other such that the S material portions tend to be more solvated by the carrier while the D material portions tend to be more dispersed in the carrier, and wherein one or more of the D material portions comprises one or more crystallizable, polymerizable compounds; and
- b) mixing the organosol with one or more additives under conditions effective to form a dispersion.

16. The method according to claim 15, wherein the step of mixing the organosol with one or more additives comprises mixing the organosol with one or more visual enhancement additives.

17. The method according to claim 16, wherein the step of mixing the organosol with one or more visual enhancement additives comprises mixing the organosol with one or more pigments.

18. The method according to claim 15, wherein the step of mixing the organosol with one or more additives comprises mixing the organosol with at least one charge control agent.

19. The method according to claim 17, wherein the step of mixing the organosol with one or more additives comprises mixing the organosol with at least one charge control agent.

20. A method of making a liquid electrographic toner composition comprising steps of:

- a) providing an organosol comprising a plurality of toner particles dispersed in a liquid carrier, wherein the toner particles comprise at least one amphipathic copolymer comprising one or more S material portions and one or more D material portions, wherein the S material portions and the D material portions have respective solubilities in the liquid carrier that are sufficiently different from each other such that the S material portions tend to be more solvated by the carrier while the D material portions tend to be more dispersed in the carrier, and wherein the D material portion has a glass transition temperature calculated according to the Fox equation of greater than 55° C., and wherein one or more polymerizable, crystallizable compounds is chemically incorporated into the D material portion, or both the S material portion and D material portion; and
- b) mixing the organosol with one or more additives under conditions effective to form a dispersion.

21. A method of electrographically forming an image on a substrate surface comprising steps of:

- a) providing a liquid toner composition, the liquid toner composition comprising an organosol, wherein the organosol comprises a plurality of toner particles dispersed in a liquid carrier, wherein the toner particles comprise at least one amphipathic copolymer comprising one or more S material portions and one or more D material portions, wherein the S material portions and the D material portions have respective solubilities in the liquid carrier that are sufficiently different from each other such that the S material portions tend to be more solvated by the carrier while the D material portions tend to be more dispersed in the carrier, wherein one or more polymerizable, crystallizable compounds is chemically incorporated into the D material portion or both the S material portion and the D material portion; and

- b) causing an image comprising the toner particles to be formed on the substrate surface.

22. The method according to claim 21 wherein the step of providing a liquid toner composition comprises providing a liquid toner composition comprising an organosol, wherein the organosol comprises a plurality of toner particles dispersed in a liquid carrier, wherein the toner particles comprise at least one visual enhancement additive and at least one amphipathic copolymer.

23. A method of electrophotographically forming an image on a substrate surface comprising steps of:

- a) providing a liquid toner composition, the liquid toner composition comprising an organosol, wherein the

**45**

organosol comprises a plurality of toner particles dispersed in a liquid carrier, wherein the toner particles comprise at least one amphipathic copolymer comprising one or more S material portions and one or more D material portions, wherein the S material portions and the D material portions have respective solubilities in the liquid carrier that are sufficiently different from each other such that the S material portions tend to be more solvated by the carrier while the D material portions tend to be more dispersed in the carrier, and wherein one or more polymerizable, crystallizable compounds is chemically incorporated into the D material portion or both the S material portion and the D material portion;

- 10 b) causing an image comprising the toner composition to be formed on a charged surface; and
- c) transferring the image from the charged surface to the substrate surface.

**24.** The method according to claim **23**, wherein the step of providing a liquid toner composition comprises providing a liquid toner composition comprising an organosol, wherein the organosol comprises a plurality of toner particles dispersed in a liquid carrier, wherein the toner particles comprise at least one visual enhancement additive and at least one amphipathic copolymer.

**25.** A method of electrophotographically forming an image on a substrate surface comprising steps of:
 

- a) providing a liquid toner composition comprising a plurality of toner particles dispersed in a liquid carrier, wherein the toner particles comprise at least one amphipathic copolymer comprising one or more S material portions and one or more D material portions, wherein the S material portions and the D material portions have respective solubilities in the liquid carrier that are sufficiently different from each other such that the S

5

10

15

20

25

30

**46**

material portions tend to be more solvated by the carrier while the D material portions tend to be more dispersed in the carrier, and wherein the D material portion has a glass transition temperature calculated according to the Fox equation of greater than 55° C., and wherein one or more polymerizable, crystallizable compounds is chemically incorporated into the D material portion, or both the S material portion and D material portion;

- b) causing an image comprising the toner composition to be formed on a charged photoreceptor surface; and, without film-forming the toner composition,
- c) transferring the image from the charged photoreceptor surface to the substrate surface.

**26.** The method according to claim **25** wherein the step of providing a liquid toner composition comprises providing a liquid toner composition comprising an organosol, wherein the organosol comprises a plurality of toner particles dispersed in a liquid carrier, wherein the toner particles comprise at least one visual enhancement additive and at least one amphipathic copolymer.

**27.** The method according to claim **25**, wherein an electrostatic potential is applied to the toner composition effect transfer from the charged photoreceptor surface to the substrate surface.

**28.** The liquid electrophotographic toner composition according to claim **1** wherein one or more polymerizable, crystallizable compounds are located in the S portion of the copolymer.

**29.** The method according to claim **15** wherein one or more of the S material portions comprises one or more crystallizable, polymerizable compounds.

\* \* \* \* \*